



US006489086B1

(12) **United States Patent**  
Kamosaki et al.

(10) **Patent No.:** **US 6,489,086 B1**  
(45) **Date of Patent:** **Dec. 3, 2002**

(54) **SILVER HALIDE COLOR PHOTOGRAPHIC PHOTOSENSITIVE MATERIAL AND METHOD FOR FORMING IMAGE**

(75) Inventors: **Tetsu Kamosaki**, Minami-Ashigara (JP); **Keizo Kimura**, Minami-Ashigara (JP); **Masashi Ogiyama**, Minami-Ashigara (JP)

(73) Assignee: **Fuji Photo Film Co., Ltd.**, Kanagawa (JP)

(\*) Notice: Subject to any disclaimer, the term of this patent is extended or adjusted under 35 U.S.C. 154(b) by 0 days.

(21) Appl. No.: **09/527,918**

(22) Filed: **Mar. 17, 2000**

(30) **Foreign Application Priority Data**

Mar. 18, 1999 (JP) ..... 11-074525

(51) **Int. Cl.**<sup>7</sup> ..... **G03C 8/40**; G03C 1/83

(52) **U.S. Cl.** ..... **430/350**; 430/383; 430/405; 430/510; 430/513; 430/516; 430/517; 430/543; 430/566

(58) **Field of Search** ..... 430/512, 513, 430/510, 517, 203, 507, 543, 559, 530, 505, 566, 350, 383, 405, 516

(56) **References Cited**

U.S. PATENT DOCUMENTS

5,756,275 A 5/1998 Takizawa et al.  
5,776,664 A 7/1998 Yamashita et al.  
6,051,359 A \* 4/2000 Ohkawa et al. ..... 430/203

6,066,440 A \* 5/2000 Araki et al. ..... 430/354  
6,337,177 B1 \* 1/2001 Kikuchi ..... 430/506

FOREIGN PATENT DOCUMENTS

|    |            |        |
|----|------------|--------|
| EP | 0276566 A1 | 8/1988 |
| EP | 0704759 A2 | 4/1996 |
| EP | 0731380 A1 | 9/1996 |
| EP | 0846982 A2 | 6/1998 |

OTHER PUBLICATIONS

Patent Abstracts of Japan—Publication No. 01167838A, Publication Date Jul. 3, 1989; vol. 013; No. 438 (Abstract).

\* cited by examiner

Primary Examiner—Thorl Chea

(74) Attorney, Agent, or Firm—Birch, Stewart, Kolasch & Birch, LLP

(57) **ABSTRACT**

Disclosed are an improved silver halide color photographic photosensitive material comprising a support having thereon a photosensitive layer containing at least one kind of photosensitive silver halide grain, a color developing agent, a coupler and a binder, and a non-photosensitive layer, wherein a one dye is contained as a dispersion of solid fine particles at least one of the layers the dye being represented by general formula (I) as follows:

D-(X)<sub>y</sub> General formula (I)

wherein D represents a compound having a chromophore; X represents a dissociative proton or a group having a dissociative proton which is linked to D directly or via a divalent linking group; and y represents an integer of 1 to 7.

**7 Claims, No Drawings**

**SILVER HALIDE COLOR PHOTOGRAPHIC  
PHOTOSENSITIVE MATERIAL AND  
METHOD FOR FORMING IMAGE**

**BACKGROUND OF THE INVENTION**

**1. Field of the Invention**

The present invention relates to a silver halide color photographic photosensitive material which enables rapid image formation. More specifically, the present invention relates to a silver halide color photographic photosensitive material which produces an image excellent in color separation and sharpness even by simple and rapid developing processing and has excellent storage stability as a product.

**2. Description of the Related Art**

Despite the advantage that a very fine image can be obtained, a silver halide color photographic photosensitive material is associated with the disadvantage that, since its development is conducted by using a processing solution having a complicated composition, the processing is subject to environmental restrictions and the control of the solution is complicated. In recent years, a dye transfer-type photosensitive material based on heat development, which dispenses with a developing solution and enables a high-quality image to be produced by using a small amount of water and heat, and an image forming apparatus using this type of photosensitive material have been developed and have become commercially available (such as "Pictography" 2000, 3000 and 4000, and "Pictrostat" 100 and 200 manufactured by Fuji Photo Film Co., Ltd.). Further, silver salt diffusion transfer-type photosensitive materials based on heat development are described in Japanese Patent Application Laid-Open (JP-A) Nos. 62-283,332; 63-198,050 and others. These systems are intended to provide, by simple heat development, print images for visual appreciation. Although heat development systems similar to those described above have been limited to photosensitive materials for the above-mentioned prints, JP-A No. 9-146,247 discloses a method for preparing a recording material for photography by a heat development system. The term "recording material for photography" as used herein means a color negative for photography, an intermediate material for plate making, and the like.

Meanwhile, in silver salt photosensitive materials for use in photography requiring high-quality images, colloidal silver or filter dye has been normally used for the purpose of improvement of color separation and sharpness. In a case where a photosensitive material for heat development is used as a recording material for photography, colloidal silver or filter dye is also necessary.

However, it is difficult to incorporate colloidal silver into a photosensitive material for heat development in which bleaching and fixing treatments are conducted using a small amount of water and processing materials. Furthermore, since colloidal silver becomes the nuclei for fog formation, the colloidal silver needs to be separated from a silver halide emulsion layer. Because of this, the film thickness increases due to the formation of an intermediate layer and the like, thus undesirably diminishing the effect of improvement of sharpness to be brought about.

The filter dye employed in the prior art is a dye which is eluted into a processing solution or decolorized at the time of developing processing. The decolorization of such a filter dye, however, is insufficient when used in photosensitive materials for heat development in which only a small amount of water is used and no developing solution is used.

As a result, the insufficiently decolorized filter dye undesirably remains as an unnecessary density component when image information is read from the photosensitive material after heat development.

5 Further, in the heat development system which is conducted by supplying a small amount of water to the photosensitive material, if a water-soluble dye is used, the dye is eluted into the small amount of water to thereby contaminate the water. This phenomenon causes a problem that the water 10 cannot be used repeatedly. In order to solve this problem, JP-A No. 6-337,511 discloses an image forming method wherein the photosensitive material contains a water-insoluble organic pigment in a state of a dispersion of solid fine particles so that heat development is conducted in the 15 presence of water. This method is still associated with a problem that the pigment may remain as an unnecessary density component.

In order to solve these problems, JP-A No. 8-101,487 discloses an image forming method wherein a dye in a state 20 of a solid dispersion is used. This method is likely to present a problem that, since part of the dye becomes soluble and is transferred during the storage of the photosensitive material, the reactivity between the coupler and color development agent is reduced.

25 Furthermore, JP-A No. 9-146,247 discloses a system wherein a color forming substance, composed of a leuco dye and a color developer, is decolorized by an alkali at the time of developing processing. This system, though excellent in decolorizing property, requires use of a large amount of the 30 color developer and alkali to be consumed accordingly and therefore often reduces the reactivity between the coupler and color development agent.

35 As dyes capable of solving the above-mentioned problems, JP-A Nos. 10-207,030 and 10-207,027 (corresponding to European Patent No. 0846982A2) disclose dyes which are decolorized by simple heat developing processing. However, there is no mention in these documents that the objectives of providing the photosensitive 40 material with both decolorizing property in heat development and of preserving the improvement in color separation and sharpness when a photosensitive material incorporating a color developing agent and a coupler is stored (this preservation is hereinafter referred to as "storage stability 45 before use" upon occasion) are effectively achieved by the incorporation of these dyes as a dispersion of solid fine particles into the photosensitive material.

**SUMMARY OF THE INVENTION**

50 It is, accordingly, the object of the present invention to provide a silver halide color photographic photosensitive material incorporating a color developing agent and a coupler, characterized by excellent dye decolorizing property in a simple developing processing and absence of unnecessary remaining color components when image information is read and also by excellent color separation and sharpness even after a period of storage, and to provide an image forming method.

55 The above-mentioned object has been accomplished by the present invention described below.

According to one aspect of the present invention, there is provided a silver halide color photographic photosensitive material comprising a support having thereon a photosensitive layer containing photosensitive silver halide grains, a color developing agent, a coupler and a binder, and a non-photosensitive layer, wherein a dye is contained as a 60 65

dispersion of solid fine particles in at least one of the layers, the dye being represented by general formula (I) as follows:

D-(X),

General formula (I)

wherein D represents a compound having a chromophore; X represents a dissociative proton or a group having a dissociative proton which is linked to D directly or via a divalent linking group; and y represents an integer of 1 to 7.

According to another aspect of the present invention, there is provided a silver halide color photographic photosensitive material, wherein the dye represented by the general formula (I) is a compound represented by a general formula selected from the group consisting of (I-1) to (I-6):

 $A^1=L^1-(L^2=L^3)_m-Q$ 

General formula (I-1)

 $A^1=N-Q$ 

General formula (I-2)

 $A^1=L^1-(L^2=L^3)_n-A^2$ 

General formula (I-3)

 $B^1=L^1-(L^2=L^3)_p-B^2$ 

General formula (I-4)

 $A^1=L^1-(L^2=L^3)_q-B^1$ 

General formula (I-5)

 $B^2-(L^2=L^3)_r-Q$ 

General formula (I-6)

wherein  $A^1$  and  $A^2$  each represents an acidic nucleus;  $B^1$  represents a basic nucleus;  $B^2$  represents an onium form of a basic nucleus; Q represents an aryl or heterocyclic group;  $L^1$ ,  $L^2$  and  $L^3$  each represents a methine group; m represents an integer selected from the group consisting of 0, 1 and 2; n and q each represents an integer selected from the group consisting of 0, 1, 2 and 3; p represents an integer selected from the group consisting of 0, 1, 2, 3 and 4; and r represents an integer selected from the group consisting of 1 and 2.

According to another aspect of the present invention, there is provided a silver halide color photographic photosensitive material, wherein the dye represented by the general formula (I) is an antihalation dye represented by a general formula selected from the group consisting of (I-7) and (I-8):

General formula (I-7)



General formula (I-8)



wherein  $A^{21}$  and  $A^{31}$  each represents an acidic nucleus;  $L^{21}$ ,  $L^{22}$  and  $L^{23}$  each represents a methine group;  $R^{21}$ ,  $R^{22}$ ,  $R^{31}$  and  $R^{32}$  each represents an alkyl or aryl group;  $R^{23}$ ,  $R^{24}$ ,  $R^{25}$ ,  $R^{26}$ ,  $R^{33}$ ,  $R^{34}$ ,  $R^{35}$  and  $R^{36}$  each represents a hydrogen atom or a substituent group; and r represents an integer selected from the group consisting of 0, 1 and 2, wherein  $R^{23}$  and  $R^{24}$ ,  $R^2$  and  $R^{23}$ ,  $R^{21}$  and  $R^{22}$ ,  $R^{22}$  and  $R^{23}$ ,  $R^{25}$  and  $R^{26}$ ,  $R^{33}$  and  $R^{34}$ ,  $R^{31}$  and  $R^{33}$ ,  $R^{31}$  and  $R^{32}$ ,  $R^{32}$  and  $R^{35}$ , and  $R^{35}$  and  $R^{36}$  are joinable for forming a ring.

According to another aspect of the present invention, there is provided a silver halide color photographic photo-

sensitive material, wherein the photosensitive layer and the non-photosensitive layer have a combined thickness of at least 15  $\mu$ m.

According to another aspect of the present invention, there is provided a silver halide color photographic photosensitive material, wherein at least one of the layers contains a basic metal compound poorly soluble in water.

According to another aspect of the present invention, there is provided a method of forming an image comprising the steps of:

- 10 (a) disposing on a support a photosensitive layer containing photosensitive silver halide grains, a color developing agent, a coupler and a binder;
- (b) further disposing on the support a non-photosensitive layer;
- (c) providing a dye as a dispersion of solid fine particles in at least one of the layers;
- (d) providing a basic metal compound poorly soluble in water in at least one of the layers;
- (e) providing a processing material having processing layer containing a compound capable of performing a complex forming reaction with a metal ion resulting from said basic metal compound;
- (f) placing the processing material together with the photosensitive layer thereon facing the processing layer;
- (g) swelling the layers by adding water, wherein the amount of water ranges from the minimum amount required for maximum swelling, excluding layers that function only as backing, to  $1/10$  of said minimum; and
- (h) heating from 1 to 120 seconds to achieve a temperature ranging from 50 to 100 degrees C. in the photosensitive layer and processing layer.

In a photosensitive material, such as the silver halide color photographic photosensitive material (hereinafter referred to simply as "photosensitive material" upon occasion), suited for use as a recording material for photography, the silver halide emulsion layer as a photosensitive layer and other layers are generally and often colored in order to allow these layers to absorb light of a specific wavelength range.

When it is required to control the spectral composition of the light incident on a photographic emulsion layer, it is a common practice to form a colored layer on the far side from the support relative to the silver halide emulsion layer. Such a colored layer is called filter layer. If a plurality of silver halide emulsion layers exist, the filter layer may be positioned between these emulsion layers.

In order to prevent image fogging or halation, which is based on that the rays of light, in the process of passing through the silver halide emulsion layer (hereinafter referred to simply as "emulsion layer" upon occasion) or scattered after passing through the emulsion layer, are reflected by the interface between the emulsion layer and the support or by the surface of the photosensitive material opposite to the emulsion side so that these rays of light fall again on the silver halide layer, a colored layer called antihalation layer is formed between the silver halide emulsion layer and the support or on the surface of the support on the side opposite to the silver halide emulsion layer. If a plurality of silver halide emulsion layers exist, the antihalation layer may be positioned between these layers.

In order to prevent the degradation of image sharpness, which is based on the scattering of rays of light in the silver halide emulsion layer (this phenomenon is generally called "irradiation"), the emulsion layer may also be colored.

Normally, a dye is incorporated into these layers to be colored and the dye to be incorporated for this purpose needs to meet the following requirements.

- (1) The dye should exhibit proper spectral absorption in accordance with the purpose of use.

(2) The dye should be inert in terms of photographic chemistry.

That is, the dye should not exert any chemically adverse influence, such as reduction in sensitivity, latent image regression or fogging, on the performance of the silver halide emulsion layer.

(3) The dye should be decolorized in the heat development process and should not leave any unnecessary coloration after the heat developing processing.

(4) The dye should not be diffused from the colored layer to other layer.

(5) The dye should be stable with the passage of time within a photosensitive material or in a solution and should not change color or fade.

It has been found that the dye represented by the general formula (I) is effective as a dye that meets the above-mentioned requirements.

In the present invention, it is more effective that the photosensitive layer and the non-photosensitive layer formed on the support have a total thickness of at least 15  $\mu\text{m}$  (upper limit being preferably 30  $\mu\text{m}$ ) from the standpoint of use for a recording material for photography whose thickness is relatively larger than that of a material for color print.

#### DETAILED DESCRIPTION OF THE INVENTION

Details of the present invention are described below.

First, the details of the dyes featuring the present invention and represented by the general formula (I) are given below.

A compound having a chromophore represented by D in the general formula (I) can be selected from many of known dye compounds. Examples of the compound include oxonol dyes, merocyanine dyes, cyanine dyes, styryl dyes, arylidene dyes, azomethine dyes, triphenylmethane dyes, azo dyes, anthraquinone dyes, indoaniline dyes, and so on.

The group, which is represented by X and is a dissociative proton or a group having a dissociative proton, is non-dissociative in the condition where the compound represented by the general formula (I) is incorporated in the silver halide photographic photosensitive material to thereby render the compound represented by the general formula (I) substantially water-insoluble, but is dissociative in the process where the silver halide photographic photosensitive material is developed to thereby render the compound represented by the general formula (I) substantially water-soluble. Examples of the group represented by X include carboxyl groups, sulfonamide groups, unsubstituted sulfamoyl groups, alkylsulfamoyl groups, arylsulfamoyl groups, sulfonylcarbamoyl groups, carbonylsulfamoyl groups, enol groups of oxonol dyes, phenolic hydroxyl groups, and so on.

The divalent linking group between X and D is an alkylene group, an arylene group, a heterocyclic group residue,  $-\text{CO}-$ ,  $-\text{SO}_n-$  (where n is 0, 1 or 2),  $-\text{NR}-$  (where R is a hydrogen atom, an alkyl group or an aryl group),  $-\text{O}-$ , or a divalent group composed of a combination of these linking groups. These groups may further have substituent groups such as an alkyl group, an aryl group, an alkoxy group, an amino group, an acyl group, an acylamino group, a halogen atom, a hydroxyl group, a carboxyl group, a sulfamoyl group, a carbamoyl group, a sulfonamide group, and the like. Preferred examples include  $-(\text{CH}_2)_n-$  (where n is 1, 2 or 3),  $-\text{CH}_2\text{CH}(\text{CH}_3)\text{CH}_2-$ , 1,2-phenylene, 5-carboxy-1,3-phenylene, 1,4-phenylene, 6-methoxy-1,3-phenylene,  $-\text{CONHC}_6\text{H}_4-$ , and the like.

y is preferably an integer of 1 to 5, and more preferably an integer of 1 to 3.

Among the compounds represented by the general formula (I), more preferred are compounds represented by a general formulae selected from the group consisting of (I-1) to (I-6).

|                                                              |                       |
|--------------------------------------------------------------|-----------------------|
| $\text{A}^1=\text{L}^1-(\text{L}^2=\text{L}^3)_m-\text{Q}$   | General formula (I-1) |
| $\text{A}^1=\text{N}-\text{Q}$                               | General formula (I-2) |
| $\text{A}^1=\text{L}^1-(\text{L}^2=\text{L}^3)_n-\text{A}^2$ | General formula (I-3) |
| $\text{B}^1=\text{L}^1-(\text{L}^2=\text{L}^3)_p-\text{B}^2$ | General formula (I-4) |
| $\text{A}^1=\text{L}^1-(\text{L}^2=\text{L}^3)_q-\text{B}^1$ | General formula (I-5) |
| $\text{B}^2-(\text{L}^2=\text{L}^3)_r-\text{Q}$              | General formula (I-6) |

wherein  $\text{A}^1$  and  $\text{A}^2$  each represents an acidic nucleus;  $\text{B}^2$  represents a basic nucleus;  $\text{Q}$  represents an aryl or heterocyclic group;  $\text{L}^1$ ,  $\text{L}^2$  and  $\text{L}^3$  each represents a methine group;  $m$  represents an integer selected from the group consisting of 0, 1 and 2;  $n$  and  $q$  each represents an integer selected from the group consisting of 0, 1, 2 and 3;  $p$  represents an integer selected from the group consisting of 0, 1, 2, 3 and 4; and  $r$  represents an integer selected from the group consisting of 1 and 2, with the proviso that the compound represented by any one of the formulae (I-1) to (I-6) has in the molecule at least one dissociative group selected from the group consisting of carboxyl groups, sulfonamide groups, arylsulfamoyl groups, sulfonylcarbamoyl groups, carbonylsulfamoyl groups, enol groups of oxonol dyes and phenolic hydroxyl groups and does not have other water-soluble group (e.g., sulfo group, phosphate group, and the like).

The acidic nucleus represented by  $\text{A}^1$  or  $\text{A}^2$  is preferably a cyclic ketomethylene compound or a compound having a methylene group sandwiched between electron-attractive groups.

Examples of the cyclic ketomethylene compound include 2-pyrazoline-5-one, rhodanine, hydantoin, thiohydantoin, 2,4-oxazoline-dione, iso-oxazoline, barbituric acid, thiobarbituric acid, indandione, dioxopyrazolopyridine, hydroxypyridine, pyrazolidine-dione, 2,5-dihydrofuran-2-one, pyrrolidine-2-one, and so on. These compounds may each have a substituent group.

Examples of the compound having a methylene group sandwiched between electron-attractive groups can be represented by  $\text{Z}^1\text{CH}_2\text{Z}^2$  where  $\text{Z}^1$  and  $\text{Z}^2$  each represents  $-\text{CN}$ ,  $-\text{SO}_2\text{R}^1$ ,  $-\text{COR}^1$ ,  $-\text{COOR}^2$ ,  $-\text{CONR}^1\text{R}^2$ ,  $-\text{SO}_2\text{R}^1\text{R}^2$ , or  $-\text{C}=[\text{C}(\text{CN})_2]\text{R}^1$ , or  $-\text{C}=[\text{C}(\text{CN})_2]\text{NHR}^1$ .  $\text{R}^1$  represents an alkyl group, an aryl group or a heterocyclic group, and  $\text{R}^2$  represents a hydrogen atom or the same group as  $\text{R}^1$ .  $\text{R}^1$  and  $\text{R}^2$  may each have a substituent group.

Examples of the basic nucleus represented by  $\text{B}^1$  include pyridine, quinoline, indolenine, oxazole, imidazole, thiazole, benzoxazole, benzimidazole, benzothiazole, oxazoline, naphthoxazole, pyrrole, and so on. These compounds may each have a substituent group.

$\text{B}^2$  is an onium form of a basic nucleus and examples of the onium form include the onium forms illustrative of  $\text{B}^1$ .

Examples of the aryl group represented by Q include phenyl groups and naphthyl groups. These groups may each have a substituent group (preferably an electron-donative group). The most preferred are phenyl groups substituted by an alkyl group, a dialkylamino group, a hydroxyl group, and/or an alkoxy group.

Examples of the heterocyclic groups represented by Q include pyrrole, indole, furan, thiophene, imidazole,

pyrazole, indolidine, quinone, carbazole, phenothiazine, phenoxazine, indoline, thiazole, pyridine, pyridazine, thiadiazine, pyran, thiopyran, oxadiazole, benzoquinoline, thiadiazole, pyrrolothiazole, pyrrolopyridazine, tetrazole, oxazole, coumarin, and coumarone. These may each have a substituent group.

The methine groups represented by  $L^1$ ,  $L^2$  and  $L^3$  may each have a substituent group. These substituent groups may join together to form a 5- or 6-membered ring (e.g., cyclopentene, cyclohexene and the like).

The substituent groups which may be borne by the above-mentioned groups are not particularly limited unless these substituent groups allow the compound represented by any one of the formulae (I-1) to (I-6) to substantially dissolve in water having a pH value of 5 to 7. Examples of the substituent groups include a carboxyl group, a sulfonamide group having 1 to 10 carbon atoms (e.g., a methanesulfonamide, benzenesulfonamide, butanesulfonamide, or n-octanesulfonamide group), a sulfamoyl group having 0 to 10 carbon atoms (e.g., an unsubstituted sulfamoyl, methylsulfamoyl, phenylsulfamoyl, or butylsulfamoyl group), a sulfonylcarbamoyl group having 2 to 10 carbon atoms (e.g., a methanesulfonylcarbamoyl, propanesulfonylcarbamoyl, or benzenesulfonylcarbamoyl group), an acylsulfamoyl group having 1 to 10 carbon atoms (e.g., an acetylsulfamoyl, propionylsulfamoyl, pivaloylsulfamoyl, or benzoylsulfamoyl group), a straight-chain or cyclic alkyl group having 1 to 8 carbon atoms (e.g., a methyl, ethyl, isopropyl, butyl, cyclopropyl, cyclohexyl, 2-hydroxyethyl, 4-carboxybutyl, 2-methoxyethyl, benzyl, phenethyl, 4-carboxybenzyl, or 2-diethylaminoethyl group), an alkenyl group having 2 to 8 carbon atoms (e.g., a vinyl or allyl group), an alkoxy group having 1 to 8 carbon atoms (e.g., a methoxy, ethoxy, or butoxy group), a halogen atom (e.g., F, Cl, or Br atom), an amino group having 0 to 10 carbon atoms (e.g., an unsubstituted amino, dimethylamino, diethylamino, or carboxyethylamino group), an ester group having 2 to 10 carbon atoms (e.g., a methoxycarbonyl group), an amide group having 1 to 10 carbon atoms (e.g., an acetamide or benzamide group), a carbamoyl group having 1 to 10 carbon atoms (e.g., an unsubstituted carbamoyl, methylcarbamoyl, or ethylcarbamoyl group), an aryl group having 6 to 10 carbon atoms (e.g., a phenyl, naphthyl, 4-carboxyphenyl, 3-carboxyphenyl, 3,5-dicarboxyphenyl, 4-methanesulfonamidephenyl, or 4-butanesulfonamidephenyl group), an aryloxy group having 6 to 10 carbon atoms (e.g., a phenoxy, 4-carboxyphenoxy, 3-methylphenoxy, or naphthoxy group), an alkylthio group having 1 to 8 carbon atoms (e.g., a methylthio, ethylthio, octylthio group), an arylthio group having 6 to 10 carbon atoms (e.g., a phenylthio or naphthylthio group), an acyl group having 1 to 10 carbon atoms (e.g., an acetyl, benzoyl, or propanoyl group), a sulfonyl group having 1 to 10 carbon atoms (e.g., a methanesulfonyl or benzenesulfonyl group), a ureido group having 1 to 10 carbon atoms (e.g., a ureido or methylureido group), a urethane group having 2 to 10 carbon atoms (e.g., a methoxycaronylamino or ethoxycarbonylamino group), a cyano group, a hydroxyl group, a nitro group, a heterocyclic group (e.g., a 5-carboxybenzoxazole, pyridine, sulfolane, furan, pyrrole, pyrrolidine, morpholine, piperazine, or pyrimidine ring).

The antihalation layer may contain dyes represented by the general formula (I) and having various hues in accordance with wavelengths of light for exposure. Among these compounds, preferred is the compound represented by any

one of the formulae (I-1) to (I-6), more preferred is the compound represented by the formula (I-1), (I-2), (I-3) or (I-4), and the most preferred is the compound represented by the formula (I-1) or (I-2). The compound represented by the general formula (I-1) is generally called arylidene dye while the compound represented by the general formula (I-2) is generally called azomethine dye. In addition, if the dye represented by the general formula (I-1) is an antihalation dye, the dye is preferably a compound represented by a general formula selected from the group consisting of (I-7) and (I-8).



wherein  $A^{21}$  and  $A^{31}$  each represents an acidic nucleus;  $L^{21}$ ,  $L^{22}$  and  $L^{23}$  each represents a methine group;  $R^{21}$ ,  $R^{22}$ ,  $R^{31}$  and  $R^{32}$  each represents an alkyl or aryl group;  $R^{23}$ ,  $R^{24}$ ,  $R^{25}$ ,  $R^{26}$ ,  $R^{33}$ ,  $R^{34}$ ,  $R^{35}$  and  $R^{36}$  each represents a hydrogen atom or a substituent group; and  $r$  represents an integer selected from the group consisting of 0, 1 and 2, wherein  $R^{23}$  and  $R^{24}$ ,  $R^{21}$  and  $R^{23}$ ,  $R^{21}$  and  $R^{22}$ ,  $R^{22}$  and  $R^{25}$ ,  $R^{25}$  and  $R^{26}$ ,  $R^{33}$  and  $R^{34}$ ,  $R^{31}$  and  $R^{33}$ ,  $R^{31}$  and  $R^{32}$ ,  $R^{32}$  and  $R^{35}$ , and  $R^{35}$  and  $R^{36}$  are joinable for forming a ring.

The general formulae (I-7) and (I-8) are explained in detail below.  $A^{21}$  and  $A^{31}$  each represent an acidic nucleus and are the same as  $A^1$  in the general formula (I-1). Preferably,  $A^{21}$  and  $A^{31}$  are each 2-pyrazoline-5-one, isoxazoline, hydroxypyridine, pyrazolidine-dione, or barbituric acid. More preferably,  $A^{21}$  and  $A^{31}$  are each hydroxypyridine or barbituric acid. Most preferably,  $A^{21}$  and  $A^{31}$  are each hydroxypyridine.

In the general formulae (I-7) and (I-8),  $L^{21}$ ,  $L^{22}$  and  $L^{23}$  each represent a methine group like  $L^1$ ,  $L^2$  and  $L^3$  in the general formula (I-1). Preferably, the methine group represented by  $L^{21}$ ,  $L^{22}$  or  $L^{23}$  is represented by  $=CR^{27}$ —(where  $R^{27}$  is an alkyl group having 1 to 10 carbon atoms or a hydrogen atom). As to the combination of  $L^{21}$ ,  $L^{22}$  and  $L^{23}$ , preferably  $R^{27}$  is a hydrogen atom in all of  $L^{21}$ ,  $L^{22}$  and  $L^{23}$ , or alternatively,  $R^{27}$  is a hydrogen atom in  $L^{21}$  and  $L^{23}$  while  $R^{27}$  in  $L^{22}$  is a methyl group. Most preferably,  $R^{27}$  is a hydrogen atom in  $L^{21}$ ,  $L^{22}$  and  $L^{23}$ .

In the general formulae (I-7) and (I-8),  $R^{21}$ ,  $R^{22}$ ,  $R^{31}$  and  $R^{32}$  each represents an alkyl or aryl group which may be substituted by an alkyl group, an alkenyl group, an alkynyl group, an aryl group, a hydroxyl group, a nitro group, a cyano group, a halogen atom, or a substituent group composed of an oxygen, nitrogen, sulfur or carbon atom, with the proviso that the carbon atoms of  $R^{21}$ ,  $R^{22}$ ,  $R^{31}$  and  $R^{32}$ , which carbon atoms are directly linked to the nitrogen atom in the general formulae (I-7) and (I-8), preferably have no elements other than two elements, namely hydrogen or carbon, if  $R^{21}$ ,  $R^{22}$ ,  $R^{31}$  and  $R^{32}$  are each an alkyl group. The alkyl group is a straight-chain, branched, or cyclic alkyl

group having 1 to 15 carbon atoms, preferably 1 to 5 carbon atoms, e. g., a methyl, ethyl, propyl, isopropyl, butyl, isobutyl, t-butyl, 2-methanesulfonamidoethyl, 2-hydroxylethyl, cyclopentyl, carboxymethyl, 2-carboxyethyl, 2,3-dicarboxypropyl, 3-methanesulfonylcarbamoylpropyl, 2-acetamideethyl, 2-carbamoyl, or 2-carbamoylamioethyl group.

The aryl group is an aryl group having 6 to 24 carbon atoms, preferably 6 to 12 carbon atoms, e.g., a phenyl, naphthyl, 4-carboxyphenyl, 3-carboxyphenyl, 2-carboxyphenyl, or 3,5-dicarboxyphenyl group.

Preferably,  $R^{21}$ ,  $R^{22}$ ,  $R^{31}$  and  $R^{32}$  are each an alkyl group. More specifically,  $R^{21}$ ,  $R^{22}$ ,  $R^{31}$  and  $R^{32}$  are each a methyl, ethyl, propyl, isopropyl, 2-methanesulfonamidoethyl, 2-hydroxylethyl, phenyl, carboxymethyl, 2-carboxyethyl, 2,3-dicarboxypropyl, 3-methanesulfonylcarbamoylpropyl, or 2-carbamoylamioethyl group. More preferably,  $R^{21}$ ,  $R^{22}$ ,  $R^{31}$  and  $R^{32}$  are each a methyl, ethyl, propyl, carboxymethyl, 2-carboxyethyl, or 2,3-dicarboxypropyl group.

$R^{23}$ ,  $R^{24}$ ,  $R^{25}$ ,  $R^{26}$ ,  $R^{33}$ ,  $R^{34}$ ,  $R^{35}$  and  $R^{36}$  each represents a hydrogen atom or a substituent group. Examples of the substituent group include a halogen atom, an alkyl group, an aryl group, a heterocyclic group, a cyano group, a nitro group, a hydroxyl group, a carboxyl group, a sulfo group, an alkoxy group, an aryloxy group, an acylamino group, an amino group, an alkylamino group, an anilino group, a ureido group, a sulfamoylamino group, an alkylthio group, an arylthio group, an alkoxy carbonylamino group, a sulfonamide group, a carbamoyl group, a sulfamoyl group, a sulfonyl group, an alkoxy carbonyl group, a heterocycloxy group, an azo group, an acyloxy group, a carbamoyloxy group, a silyl group, a silyloxy group, an aryloxy carbonylamino group, an imido group, a heterocyclothio group, a sulfinyl group, an phosphonyl group, an aryloxy carbonyl group, and an acyl group. These groups may be substituted by an alkyl group, an alkenyl group, an alkynyl group, an aryl group, a hydroxyl group, a nitro group, a cyano group, a halogen atom, or a substituent group composed of an oxygen, nitrogen, sulfur or carbon atom.

More specific examples of the substituent groups of  $R^{23}$ ,  $R^{24}$ ,  $R^{25}$ ,  $R^{26}$ ,  $R^{33}$ ,  $R^{34}$ ,  $R^{35}$  and  $R^{36}$  are given below. Examples of the halogen atom include a fluorine atom, a chlorine atom, and so on. Examples of the alkyl group and the aryl group are the same as those listed for the explanation of  $R^{21}$ ,  $R^{22}$ ,  $R^{31}$  and  $R^{32}$ . Examples of the heterocyclic group are the same as those listed for the explanation of the substituent groups which may be borne by the compounds represented by the formulae (I-1) to (I-6).

The alkoxy group is an alkoxy group having 1 to 16 carbon atoms, preferably 1 to 3 carbon atoms, e.g., a methoxy, ethoxy, 2-methoxyethoxy, or 2-methanesulfonylethoxy group. The aryloxy group is an aryloxy group having 6 to 24 carbon atoms, preferably 6 to 8 carbon atoms, e.g., a phenoxy, p-methoxyphenoxy, or m-(3-hydroxypropionamide)phenoxy group. The acylamino group is an acylamino group having 1 to 16 carbon atoms, preferably 1 to 6 carbon atoms, e.g., an acetamide, 2-methoxypropionamide, or p-nitrobenzoylamide group.

The alkylamino group is an alkylamino group having 1 to 16 carbon atoms, preferably 1 to 4 carbon atoms, e.g., dimethylamino, diethylamino, or 2-hydroxyethylamino group. The anilino group is an anilino group having 6 to 24 carbon atoms, e.g., an m-nitroanilino or N-methylanilino group. The ureido group is a ureido group having 1 to 16 carbon atoms, preferably 1 to 6 carbon atoms, e.g., a ureido, methylureido, N,N-diethylureido, or 2-methanesulfonamidoethylureido group.

The sulfamoylamino groups is a sulfamoylamino group having 0 to 16 carbon atoms, preferably 0 to 3 carbon atoms, e.g., a dimethylsulfamoylamino, methylsulfamoylamino, or 2-methoxylethylsulfamoylamino group. The alkylthio group is an alkylthio group having 1 to 16 carbon atoms, preferably 1 to 3 carbon atoms, e.g., a methylthio, ethylthio, 2-phenoxyethylthio group. The arylthio group is an arylthio group having 6 to 22 carbon atoms, preferably 6 to 8 carbon atoms, e.g., a phenylthio, 2-carboxyphenylthio, or 4-cyanophenylthio group. The alkoxy carbonylamino group is an alkoxy carbonylamino group having 2 to 16 carbon atoms, preferably 2 to 6 carbon atoms, e.g., a methoxycarbonylamino, ethoxycarbonylamino, 3-methanesulfonylpropoxycarbonylamino group.

The sulfonamide group is a sulfonamide group having 1 to 16 carbon atoms, preferably 1 to 6 carbon atoms, e.g., a methanesulfonamide, p-toluenesulfonamide, or 2-methoxyethanesulfonamide group. The carbamoyl group is a carbamoyl group having 1 to 16 carbon atoms, preferably 1 to 6 carbon atoms, e.g., a carbamoyl, N,N-dimethylcarbamoyl, or N-ethylcarbamoyl group. The sulfamoyl groups is a sulfamoyl group having 0 to 16 carbon atoms, preferably 0 to 6 carbon atoms, e.g., a sulfamoyl, dimethylsulfamoyl, or ethylsulfamoyl group.

The sulfonyl group is an aliphatic or aromatic sulfonyl group having 1 to 16 carbon atoms, preferably 1 to 6 carbon atoms, e.g., a methanesulfonyl, ethanesulfonyl, or 2-chloroethanesulfonyl group. The alkoxy carbonyl group is an alkoxy carbonyl group having 1 to 16 carbon atoms, preferably 1 to 3 carbon atoms, e.g., a methoxycarbonyl, ethoxycarbonyl, or t-butoxycarbonyl group. The heterocycloxy group is a 5- or 6-membered, saturated or unsaturated heterocycloxy group having 1 to 5 carbon atoms and at least one oxygen, nitrogen or sulfur atom, wherein the number of the heteroatom and the kind of the element constituting the ring may be one or more, e.g., a 1-phenyltetrazolyl-5-oxy, 2-tetrahydropyranoxy, or 2-pyridyloxy group.

The azo group is an azo group having 1 to 16 carbon atoms, preferably 1 to 6 carbon atoms, e.g., a phenylazo, 2-hydroxy-4-propanoylphenylazo, 4-sulfophenylazo group. The acyloxy group is an acyloxy group having 1 to 16 carbon atoms, preferably 1 to 6 carbon atoms, e.g., an acetoxy, benzyloxy, or 4-hydroxybutanoyloxy group. The carbamoyloxy group is a carbamoyloxy group having 1 to 16 carbon atoms, preferably 1 to 6 carbon atoms, e.g., an N,N-dimethylcarbamoyloxy, N-methylcarbamoyloxy, or N-phenylcarbamoyloxy group.

The silyl group is a silyl group having 3 to 16 carbon atoms, preferably 3 to 6 carbon atoms, e.g., a trimethylsilyl, isopropylidethylsilyl, or t-butyldimethylsilyl group. The silyloxy group is a silyloxy group having 3 to 16 carbon atoms, preferably 3 to 6 carbon atoms, e.g., a trimethylsilyloxy, triethylsilyloxy, or diisopropylethylsilyloxy group. The aryloxy carbonylamino group is an aryloxy carbonylamino group having 7 to 24 carbon atoms, preferably 7 to 11 carbon atoms, e.g., a phenoxy carbonylamino, 4-cyanophenoxy carbonylamino, or 2,6-dimethoxyphenoxy carbonylamino group.

The imido group is an imido group having 4 to 16 carbon atoms, preferably 4 to 8 carbon atoms, e.g., an N-succinimido or N-phthalimide group. The heterocyclothio group is a 5- or 6-membered, saturated or unsaturated heterocyclothio group having 1 to 5 carbon atoms and at least one oxygen, nitrogen or sulfur atom, wherein the number of the heteroatom and the kind of the element constituting the ring may be one or more, e.g., a 2-benzothiazolylthio or 2-pyridylthio group.

## 11

The sulfinyl group is a sulfinyl group having 1 to 16 carbon atoms, preferably 1 to 6 carbon atoms, e.g., a methanesulfinyl, benzenesulfinyl, or ethanesulfinyl group. The phosphonyl group is a phosphonyl group having 2 to 16 carbon atoms, preferably 2 to 6 carbon atoms, e.g., a methoxyphosphonyl, ethoxyphosphonyl, or phenoxyphosphonyl group. The aryloxycarbonyl group is an aryloxycarbonyloxy group having 7 to 24 carbon atoms, preferably 7 to 11 carbon atoms, e.g., a phenoxy carbonyl, 2-methylphenoxy carbonyl, or 4-acetamidophenoxy carbonyl group. The acyl group is an acyl group having 1 to 16 carbon atoms, preferably 1 to 6 carbon atoms, e.g., an acetyl, benzoyl, or 4-chlorobenzoyl group.

Preferred examples of  $R^{23}$ ,  $R^{24}$ ,  $R^{25}$ ,  $R^{26}$ ,  $R^{33}$ ,  $R^{34}$ ,  $R^{35}$  and  $R^{36}$  include a hydrogen atom, an alkyl group, an aryl group, an alkoxy group, an acylamino group, a ureido group, a sulfamoylamino group, a sulfonylamino group, a carbamoyl group, and a sulfamoyl group. More preferably,  $R^{23}$ ,  $R^{24}$ ,  $R^{25}$ ,  $R^{26}$ ,  $R^{33}$ ,  $R^{34}$ ,  $R^{35}$  and  $R^{36}$  are each a hydrogen atom, an alkyl group, an alkoxy group, a carbamoyl group, a sulfamoyl group, or a ureido group, and most preferably a hydrogen atom, an alkyl group, or an alkoxy group.

Specifically, preferred examples of  $R^{23}$ ,  $R^{24}$ ,  $R^{25}$ ,  $R^{26}$ ,  $R^{33}$ ,  $R^{34}$ ,  $R^{35}$  and  $R^{36}$  include a hydrogen atom, methyl, ethyl, n-propyl, i-propyl, n-butyl, t-butyl, t-pentyl, di-t-octyl, hydroxymethyl, 1,3-dihydroxy-2-propyl, phenyl, m-hydroxyphenyl, methoxy, ethoxy, i-propoxy, 2-hydroxyethoxy, 2-methanesulfonylethoxy, acetamide, 2-methoxypropionamide, p-hydroxybenzoylamide, ureido, methylureido, N,N-dimethylureido, 2-methanesulfonamide ethylureido, dimethylsulfamoylamino, methylsulfamoylamino, 2-methoxyethylsulfamoylamino, methanesulfonamide, p-toluenesulfonamide, 2-methoxyethanesulfoneamide, carbamoyl, N,N-dimethylcarbamoyl, N-ethylcarbamoyl, sulfamoyl, dimethylsulfamoyl, and ethylsulfamoyl groups.

## 12

$R^{23}$ ,  $R^{24}$ ,  $R^{25}$ ,  $R^{26}$ ,  $R^{33}$ ,  $R^{34}$ ,  $R^{35}$  and  $R^{36}$  are more preferably a hydrogen atom, methyl, ethyl, n-propyl, i-propyl, t-butyl, methoxy, i-propoxy, acetamide, methylureido, N,N-dimethylureido, dimethylsulfamoylamino, methylsulfamoylamino, methanesulfonamide, carbamoyl, N,N-dimethylcarbamoyl, N-ethylcarbamoyl, sulfamoyl, and dimethylsulfamoyl groups, and most preferably a hydrogen atom, methyl, ethyl, i-propyl, methoxy, and i-propoxy groups.

Further,  $R^{23}$  and  $R^{24}$ ,  $R^{21}$  and  $R^{23}$ ,  $R^{21}$  and  $R^{22}$ ,  $R^{22}$  and  $R^{25}$ ,  $R^{25}$  and  $R^{26}$ ,  $R^{33}$  and  $R^{34}$ ,  $R^{31}$  and  $R^{33}$ ,  $R^{31}$  and  $R^{32}$ ,  $R^{32}$  and  $R^{35}$ , and  $R^{35}$  and  $R^{36}$  may each join together to form a ring. Furthermore, any one of  $R^{24}$  and  $R^{22}$  may form a ring together with  $L^{21}$  or  $L^{23}$ . In particular, it is preferable that any one of  $R^{21}$  and  $R^{23}$ ,  $R^{22}$  and  $R^{25}$ ,  $R^{31}$  and  $R^{33}$ ,  $R^{32}$  and  $R^{35}$  and  $R^{24}$  and  $R^{26}$  joins with  $L^{21}$  or  $L^{23}$  to form a substituted or unsubstituted ethylene or trimethylene chain. In this case, the substituent groups are the same as those listed for the explanation of  $R^{23}$ ,  $R^{24}$ ,  $R^{25}$ ,  $R^{26}$ ,  $R^{33}$ ,  $R^{34}$ ,  $R^{35}$  and  $R^{36}$ . Preferred examples of the substituent group include a hydroxy group, a halogen atom, an alkyl group, an alkoxy group, a carboxyl group, an acylamino group, an alkylamino group, a ureido group, a sulfamoylamino group, an alkoxy carbonylamino group, a sulfonylamino group, a carbamoyl group, a sulfamoyl group, a sulfonyl group, an alkoxy carbonyl group, an acyloxy group, a carbamoyloxy group, an acyl group, and so on. The substituent groups are more preferably a hydroxy group, an alkyl group, a carboxyl group, an acylamino group, a ureido group, an alkoxy carbonylamino group, a sulfamoylamino group, a carbamoyl group, an acyloxy group, and a carbamoyloxy group, and most preferably a hydroxy group, an alkyl group, and a carboxyl group.

Specific examples of the dyes represented by the general formula (I) are given below. It should be understood that the present invention is not limited to these examples.



**13****14**

-continued

F-5

F-6



F-7

F-8



F-9

F-10



F-11

F-12



15

16

-continued

F-13

F-14



F-15



F-17



F-18

F-19



17



18



-continued

F-21

F-22



F-23

F-24



F-25

F-26



F-27

F-28



F-29

F-30



**19****20**

-continued

F-31



F-32



F-33

F-34



F-35

F-36



F-37

F-38



F-39

F-40



21

22

-continued



F-43

F-42



F-45

F-46



F-47

F-48



F-49

F-50



F-51

F-52



23

24

-continued

F-53



F-54



F-55



F-56



F-57



F-58



F-59



F-60



25

26

-continued

F-61



F-62



E. 64



F-65



F-66



F-67



F-68

-continued

F-69



F-70



F-71



F-72



F-73



F-74



F-75



-continued

F-76



F-77



F-78



F-79



F-80



-continued

F-81



F-82



F-83



F-84





-continued

F-90



F-91



F-92



F-93



**37****38**

-continued

F-94



F-95



F-96



F-97



-continued

F-98



F-99



F-100



F-101

F-102



F-103

F-104



-continued

F-105

F-106



F-107

F-108



F-109

F-110



F-111

F-112



F-113

F-114



F-115

F-116



**43****44**

-continued

F-117

F-118



F-119

F-120



F-121

F-122



F-123

F-124



45

46

-continued

F-125



E 126



F-127

F-128



E-129

E-130



E 131



47



-continued

F-132



F-134



F-136



F-137



F-138

F-139



F-140



F-141

F-142



F-143



-continued

F-144



F-145



F-146



F-147



F-148

F-149



F-150



F-151



51

52

-continued

F-152

F-153



F-154



F-155



F-156

F-157



F-156

F-157

F-156



F-158

F-159

F-160

F-161



-continued

F-162



F-163



F-164

F-165



F-166

F-167



F-168

F-169



F-170

F-171



-continued

F-172



F-173



F-174



F-175



F-176



F-177



F-178



F-179



F-180



F-181

**57****58**

-continued

F-182 F-183



F-184 F-185



F-186 F-187



F-188 F-189





-continued

F-190

F-191



F-192

F-193



F-194

F-195



F-196



F-197



F-198

-continued

F-199



F-200



F-201



F-202



F-203



F-204



F-205

F-206



**63****64**

-continued

F-207



F-208



F-209



F-210



F-211



F-212



-continued



The dyes which are to be used in the present invention and are represented by the general formula (I) can be synthesized by the same or nearly the same processes as those described in International Patent WO88/04794; European Patent Application Nos. EP0274,723A1; 276,566; and 299,435; U.S. Pat. Nos. 2,527,583; 3,486,897; 3,746,539; 3,933,798; 4,130,429; 4,040,841; JP-A Nos. 48-68,623; 52-92,716; 55-155,350; 55-155,351; 61-205,934; 2-173,630; 2-230, 135; 2-277,044; 2-282,244; 3-7,931; 3-167,546; 3-13,937; 3-206,443; 3-208,047; 3-192,157; 3-216,645; 3-274,043; 4-37,841; 4-45,436; 4-138,449; 5-197,077; 6-332,112; 7-206,824; 8-20,582; and so on.

As typical examples, some specific synthetic processes for making the illustrative compounds as the dyes represented by the general formula (I) are given below.

(Synthesis-1) Synthesis of the illustrative compound F-3

The process for the synthesis of the illustrative compound F-3 is indicated by the following chemical formulae.



Steps of the process are explained below.

#### Synthesis of the Compound (2)

A three-neck flask was charged with 165 g of the compound (1), 40.4 mL of pyridine, and 500 mL of dimethylacetamide. While the reaction mixture was stirred at a liquid temperature of 83° C. on a steam bath, 126 g of diketene was added dropwise to the reaction mixture over a period of 20 minutes. After the completion of the dropwise addition, the reaction mixture was continuously heated with stirring at that temperature for additional 2 hours and thereafter cooled to room temperature. Then, 1L of ethyl acetate and 1L of water were added to the reaction mixture to extract the reaction product. The ethyl acetate layer thus obtained was washed 4 times with a solvent mixture composed of 100 mL of saturated aqueous solution of sodium chloride and 600 mL of water. The solution in ethyl acetate was dried by using anhydrous sodium sulfate and thereafter concentrated by using a rotary evaporator. In this way, the target compound (2) was obtained as a crude product. The compound (2) thus obtained as a crude product was subjected straight to the following step.

## Synthesis of the Compound (4)

A three-neck flask was charged with the compound (2) obtained in the preceding step, 102 g of piperidine, and 500 mL of isopropyl alcohol. While the reaction mixture was stirred at reflux temperature, 139 g of the compound (3) was added dropwise to the reaction mixture over a period of 20 minutes. After the completion of the dropwise addition, the reaction mixture was maintained at reflux temperature with stirring for additional 3 hours and thereafter cooled to room temperature. Then, 1L of ethyl acetate, 1L of water and 120 mL of a concentrated aqueous solution of hydrochloric acid were added to the reaction mixture to extract the reaction product. The ethyl acetate layer thus obtained was washed 4 times with a solvent mixture composed of 100 mL of saturated aqueous solution of sodium chloride and 600 mL of water. The solution in ethyl acetate was dried by using anhydrous sodium sulfate and thereafter concentrated by using a rotary evaporator. Then, 1L of acetonitrile was added to the residue thus obtained and the crystals that deposited were collected by filtration under suction. In this way, 238 g (80% yield) of the target compound (4) was obtained.

## Synthesis-of the Compound (5)

A three-neck flask was charged with 149 g of the compound (4) and 450 mL of ethanol. While the reaction mixture was stirred, a solution prepared by dissolving 80 g of sodium hydroxide in 160 mL of water was added dropwise to the

reaction mixture over a period of 5 minutes. After the completion of the dropwise addition, the reaction mixture was stirred for additional 30 minutes and thereafter poured into 1 kg of water. Then, while the reaction mixture was stirred, 257 mL of a concentrated aqueous solution of hydrochloric acid was added to the reaction mixture and the reaction mixture was stirred for one hour. After that, the crystals that deposited were collected by filtration under suction. In this way, 128 g (95% yield) of the target compound (5) was obtained. Synthesis of the illustrative compound F-3.

A three-neck flask was charged with 81 g of the compound (5), 53 g of the compound (6), and 1.2 L of methanol. The reaction mixture was stirred at reflux temperature for 30 minutes and thereafter cooled to room temperature. After that, the crystals that deposited were collected by filtration under suction. The crystals thus collected were added with 500 mL of methanol. The mixture was stirred at reflux temperature for 15 minutes and thereafter cooled to room temperature. After that, the crystals were collected by filtration under suction and were then dried. In this way, 112 g (87% yield) of the illustrative compound F-3 aimed at was obtained.

## (Synthesis-2) Synthesis of the Illustrative Compound F-81

The process for the synthesis of the illustrative compound F-81 is indicated by the following chemical formulae.



-continued



30

Steps of the process are explained below.  
Synthesis of the Compound (9)

A three-neck flask was charged with 1.2 L of ethanol and 308 g of the compound (8). While the reaction mixture was stirred at room temperature, 228 g of the compound (7) was added dropwise to the reaction mixture over a period of 10 minutes. After the completion of the dropwise addition, the reaction mixture was stirred for additional 3 hours. Then, while the reaction mixture was stirred, a solution prepared by dissolving 198 g of sodium hydroxide in 1080 mL of water was added dropwise to the reaction mixture over a period of one hour. The addition caused the interior temperature to rise to 35° C. After the completion of the dropwise addition, the reaction mixture was stirred for additional one hour and 30 minutes. After that, the reaction mixture was poured into 6 L of methanol. Subsequently, 412 mL of a concentrated aqueous solution of hydrochloric acid was added dropwise to the reaction mixture in methanol over a period of 30 minutes and the mixture was stirred for additional one hour. The crystals that deposited were collected by filtration under suction. The crystals thus collected were washed with water and then dried. In this way, 345 g (95% yield) of the target compound (9) was obtained.

Synthesis of the Compound (11)

A three-neck flask was charged with 400 mL of sulfolane. While the sulfolane was stirred under a nitrogen stream, 310 g of the compound (9) was charged into the flask and thereafter 268 g of the compound (10) was charged into the flask. The reaction mixture was then heated to a liquid temperature of 90° C., at which temperature 24.0 g of methanesulfonic acid was added dropwise to the reaction mixture over a period of 3 minutes. After the completion of the dropwise addition, the reaction mixture was stirred at 135° C. for one hour and thereafter cooled to room temperature. The reaction mixture was then added to 1.5 L of methanol with stirring. After the completion of the addition, the mixture was stirred for one hour. The crystals that deposited

were collected by filtration under suction and then dried. In this way, 404 g (88% yield) of the target compound (11) was obtained.

Synthesis of the Compound (13)

A three-neck flask was charged with 420 g of acetic acid. While the flask was cooled on an ice bath, 283 g of triethylamine was charged dropwise into the flask while the liquid temperature was kept at 50° C. or below. Further, 257 g of the compound (11) was charged into the flask and thereafter 109.3 g of the compound (12) was charged into the flask. After that, the reaction mixture was stirred at a liquid temperature of 90° C. for 5 hours and thereafter cooled to room temperature. The reaction mixture was then added to 2 L of methanol with stirring. After the completion of the addition, 292 mL of a concentrated aqueous solution of hydrochloric acid was added dropwise to the reaction mixture in methanol over a period of 30 minutes and the mixture was stirred for additional one hour. The crystals that deposited were collected by filtration under suction and then dried. In this way, 280 g (92% yield) of the target compound (13) was obtained.

Synthesis of the Compound (14)

A three-neck flask was charged with 260 g of the compound (13) and 1.2 L of ethanol. Then, while the reaction mixture was stirred, a solution prepared by dissolving 120 g of sodium hydroxide in 650 mL of water was added dropwise to the reaction mixture over a period of 30 minutes. After the completion of the dropwise addition, the reaction mixture was stirred for additional two hours. The reaction mixture was then added to 2.2 L of methanol with stirring. After the completion of the addition, 330 mL of a concentrated aqueous solution of hydrochloric acid was added dropwise to the reaction mixture in methanol over a period of 20 minutes and the mixture was stirred for additional one hour. The crystals that deposited were collected by filtration under suction and then dried. In this way, 241 g (99% yield) of the target compound (14) was obtained.

### Synthesis of the Illustrative Compound (F-81)

A three-neck flask was charged with 109.4 g of the compound (14), 56.8 g of the compound (6), and 2.2 L of acetic acid. While the reaction mixture was stirred, 193 g of acetic anhydride was charged into the flask. After that, the reaction mixture was stirred at a liquid temperature of 100° C. for 2 hours and thereafter cooled to room temperature. The crystals that deposited were collected by filtration under suction and washed with solvents, that is, acetic acid, methanol, acetone and methanol, in that order. In this way, 384 g as methanol-wet cake of the illustrative compound (F-81) aimed at was obtained. Since the dye content of the substance thus obtained was 38.3%, the yield of the reaction was 97%.

### (Synthesis-3) Synthesis of the Illustrative Compound F-118

The process for the synthesis of the illustrative compound F-118 is indicated by the following chemical formulae.

The dye represented by the general formula (I) is used as a dispersion of solid fine powder (fine crystal particles). The dispersion of solid fine (crystal) particles of dye can be prepared in a mechanical way using, if desired, a proper solvent (water, alcohol, or the like), by a known pulverizing means (e.g., ball mill, vibration ball mill, planetary ball mill, sand mill, colloid mill, jet mill, roller mill, and so on) in the presence of a dispersant. The fine (crystal) particles of dye can also be obtained, for example, by a method wherein the dye is first dissolved in a proper solvent by using a dispersant and the solution is then added to a poor solvent of the dye to thereby deposit fine crystals, or by a method wherein the dye is first dissolved by controlling pH and then are converted into fine crystals by changing the pH. A layer containing fine powder of the dye can be obtained by preparing a solid dispersion of nearly uniform particles by dispersing the fine (crystal) particles obtained above in a proper binder.



## Synthesis of the Illustrative Compound F-118

A three-neck flask was charged with 20.3 g of the compound (14) and 60 mL of methanol. While the reaction mixture was stirred at room temperature, 7.0 mL of triethylamine was added dropwise to the reaction mixture over a period of 3 minutes. After the completion of the dropwise addition, 10.0 g of the compound (15) was added and thereafter 5.2 mL of acetic anhydride was added dropwise to the reaction mixture over a period of 10 minutes. The reaction mixture was stirred for additional 4 hours at room temperature and the crystals that deposited were collected by filtration under suction. The crystals thus obtained were added with 400 mL of methanol and 100 mL of acetone and the mixture was stirred. Next, while being washed with methanol, the crystals were collected by filtration under suction. In this way, 58.0 g as methanol-containing cake of the illustrative compound F-118 was obtained. Part of the cake was dried and the dye content was found to be 48.0% (99% yield).

50 and then coating the dispersion on a desired support. Alternatively, the layer containing the fine powder of the dye can be obtained by a coating a solution composed of a salt of dissociated dye on a support and then overcoating the layer with a primer and/or topcoat having an acidity in accordance with the  $pK_a$  of the dissociative group to thereby disperse and fix the particles at the time of coating.

The binder is not particularly limited if it is a hydrophilic colloid which can be used for photosensitive layers (emulsion layers) and non-photosensitive layers. Normally, a naturally occurring polymer such as gelatin and the like or 60 a synthetic polymer is used as the binder. The substances usable as the binder are, for example, protein such as gelatin derivatives, graft polymers made up of gelatin and other polymer, albumin or casein; cellulose derivatives, such as hydroxyethylcellulose, hydroxymethylcellulose, 65 hydroxypropylcellulose, carboxymethylcellulose, ethylcellulose, methylcellulose, nitrocellulose, cellulose sulfate ester, and the like; saccharide derivatives, such as

dextrin, sodium alginate, pectin, carboxymethyl starch, and the like; gum arabic, polyalkylene oxides, polyvinyl alcohol, modified polyvinyl alcohol described in JP-A No. 7-219, 113, partially acetalized polyvinyl alcohol, polyvinyl butyral, poly-N-vinyl pyrrolidone, polyethyloxazoline, polyvinylmethyloxazoline, polyacrylic acid, polymethacrylic acid, acryloylmethylpropane/sulfonic acid copolymers, polymeric methacrylic acids such as those described in European Patent Application No. EP 678, 770A2, and synthetic polymers, such as homopolymers and copolymers, e.g., copolymers of maleic acid, esters or amides thereof, polyacrylamide, polyvinylimidazole, polyvinylpyrazole, and so on. These substances may be added at the dispersing stage.

The dispersants may be known surface active agents. Examples of the dispersants include anionic dispersants, nonionic dispersants and combinations thereof described in U.S. Pat. No. 4,060,025, JP-A Nos. 62-215,272; 1-201,655; 4-125,548, U.S. Pat. No. 5,104,776, European Patent Application No. EP678,771A2, JP-A Nos. 63-11,935 and 63-60, 446, amphoteric dispersants described in U.S. Pat. No. 3,542,581 and European Patent Application No. EP569, 074A1, and fluorine-containing dispersants described in European Patent Application No. EP602,428A1. In particular, the use of anionic dispersants and/or nonionic dispersants is preferable. The anionic dispersants described in JP-A No. 4-324,858, oligomer-type polymers described in JP-A Nos. 60-158,437 and 7-13,300, and nonionic polymers described in U.S. Pat. No. 3,860,425 can be more preferably used. These can also be added after the dispersing operation. The amount to be used of the dispersant is 1 to 200% by weight based on the amount of the dye to be dispersed.

The average particle diameter of the fine particles of the dye in the dispersion of solid particles is 0.005 to 10  $\mu\text{m}$ , preferably 0.01 to 1  $\mu\text{m}$ , and more preferably 0.01 to 0.5  $\mu\text{m}$ . It is preferably 0.01 to 0.1  $\mu\text{m}$  in some cases.

Depending on the hue of the dye, the dispersion of the fine (crystal) particles of the dye represented by the general formula (I) can be used in any of a silver halide photosensitive layer and non-photosensitive layer. In the case where the dispersion of the fine (crystal) particles of the dye is incorporated in a non-photosensitive layer of a photosensitive material, for example a color negative photosensitive material, having an antihalation layer formed between a support and a silver halide emulsion layer and a plurality of non-photosensitive layers, it is preferable that these layers are constructed such that a yellow filter layer is formed between a blue-sensitive silver halide photosensitive layer and a green-sensitive silver halide photosensitive layer; a magenta filter layer is formed between a green-sensitive silver halide photosensitive layer and red-sensitive silver halide photosensitive layer; and an antihalation layer is formed between a support and a red-sensitive silver halide photosensitive layer, and it is preferable that the dispersion of the fine (crystal) particles of the dye represented by the general formula (I) is incorporated in these non-photosensitive layers. Further, it is also possible to form a back layer on the support on the side opposite to the side having these silver halide photosensitive layers and non-photosensitive layers in order that the back layer contains the dispersion of the fine (crystal) particles of the dye represented by the general formula (I).

In the present invention, if non-photosensitive layers are formed as layers having the above-mentioned functions (such as antihalation layer, yellow filter layer, magenta filter layer, and the like), it is preferable that each of these non-photosensitive layers contains the dispersion of the fine (crystal) particles of the dye represented by the general formula (I).

In the present invention, the amount to be added of the dispersion the fine (crystal) particles of the dye represented by the general formula (I) to the photosensitive material (photosensitive layers and/or non-photosensitive layers) is in the range of from  $5.0 \times 10^{-5}$  to 5.0 g per  $\text{m}^2$  of the photosensitive material. The amount is preferably in the range of from  $5.0 \times 10^{-4}$  to 2.0 g and more preferably in the range of from  $5.0 \times 10^{-3}$  to 1.0 g per  $\text{m}^2$  of the photosensitive material. One or more kinds of the dyes may be incorporated in the same layer, or alternatively, one kind of the dye may be incorporated in a plurality of layers. Further, a known dye other than the dyes of the present invention may be used in combination, if necessary.

In the present invention, the use of the dispersion of the fine (crystal) particles of the dye represented by the general formula (I) alleviates the following problems. These problems are encountered in traditionally known processes, for example, a mordanting process wherein the dye molecule is fixed by the presence in the same layer of a hydrophilic polymer as a mordant which has an electric charge opposite to that of the dissociated anionic dye, and a process using a dispersion prepared from an oil-soluble dye finely dispersed or latex-dispersed in water or in a gelatin solution by use of an organic solvent having a high boiling point. The problems are undesirable influence on photographic properties such as reduction in sensitivity which is caused by the diffusion of dye to other layer due to insufficient fixation of the dye and image quality degradation caused by unnecessary absorption of the remaining color due to insufficient decolorization.

In the present invention, the dye represented by the general formula (I) (this dye is hereinafter referred to simply as "dye" upon occasion) is decolorized due to the reaction with a decolorizing agent when processed in the presence of the decolorizing agent.

Examples of the decolorizing agent include alcohol or phenols ( $\text{R}_{51}\text{OH}$ ), amines or anilines ( $(\text{R}_{52})_3\text{N}$ ), hydroxylamines ( $(\text{R}_{52})_2\text{NOR}_{52}$ ), sulfonic acids ( $\text{R}_{51}\text{SO}_2\text{H}$ ) or salts thereof, sulfuric acid or salts thereof, thiosulfuric acid or salts thereof, carboxylic acids ( $\text{R}_{51}\text{CO}_2\text{H}$ ) or salts thereof, hydrazines ( $(\text{R}_{52})_2\text{NN}(\text{R}_{52})_2$ ), guanidines ( $[(\text{R}_{52})_2\text{N}]_2\text{C}=\text{NH}$ ), aminoguanidines ( $(\text{R}_{52})_2\text{NR}_{52}\text{N}(\text{R}_{52})\text{C}(\text{NH})$ ), amidines, thiols ( $\text{R}_{51}\text{SH}$ ), cyclic or chain-like active methylene compounds ( $\text{Z}_{53}-\text{CH}_2-\text{Z}_{54}$ ), cyclic or chain-like methylene compounds ( $\text{Z}_{53}\text{CH}(\text{R}_{51})-\text{Z}_{54}$ ) or  $\text{Z}_{53}-\text{CH}(\text{Z}_{54})-\text{Z}_{55}$ , where  $\text{Z}_{55}$  is the same as  $\text{Z}_{53}$  and where  $\text{Z}_{53}$ ,  $\text{Z}_{54}$ , and  $\text{Z}_{55}$  (or  $\text{R}_{51}$ ) may join with each other to form a ring, and anionic species derived from these compounds.

In the compounds described above,  $\text{R}_{51}$  represents an alkyl group, an alkenyl group, a cycloalkyl group, an aryl group or a heterocyclic group, while  $\text{R}_{52}$  represents a hydrogen atom or the same group as  $\text{R}_{51}$ . Each of  $\text{R}_{51}$  and  $\text{R}_{52}$  may have a substituent group. If a plurality of  $\text{R}_{51}$  or  $\text{R}_{52}$  are present in the molecule, they may be the same or different.  $\text{Z}_{53}$  and  $\text{Z}_{54}$  are each selected from the group consisting of  $-\text{CN}$ ,  $-\text{SO}_2\text{R}_{51}$ ,  $-\text{COR}_{51}$ ,  $-\text{COOR}_{51}$ ,  $-\text{CON}(\text{R}_{52})_2$ ,  $-\text{SO}_2\text{N}(\text{R}_{52})_2$ ,  $-\text{C}=[\text{C}(\text{CN})_2]$   $\text{R}_{51}$ , and  $-\text{C}=[\text{C}(\text{CN})_2]\text{N}(\text{R}_{51})_2$  wherein  $\text{Z}_{53}$  may be the same as or different from  $\text{Z}_{54}$ , and  $\text{Z}_{53}$  and  $\text{Z}_{54}$  may join together to form a ring.

Among these compounds, preferable are hydroxylamines, sulfonic acids, sulfuric acid, guanidines, aminoguanidines, heterocyclic thiols, cyclic or chain-like active methylene compounds and active methine compounds. Particularly preferable are guanidines and aminoguanidines.

These decolorizing agents may be incorporated into photosensitive materials at the preparation thereof, or these decolorizing agents may be added to the photosensitive

materials by an appropriate method when the photosensitive materials are processed. Preferably, a processing material contains the decolorizing agent and the decolorizing agent is transferred to the photosensitive material at the time of thermal processing. When added, these decolorizing agents may be in the form of precursors.

The decolorizing agent is thought to make contact with dye molecules to undergo nucleophilic addition to the dye molecule so that the dye is decolorized when the photosensitive material is processed. As a preferable procedure, a dye-containing silver halide photosensitive material after imagewise exposure or at the time of imagewise exposure thereof is put together with a processing material, which contains a decolorizing agent or a precursor thereof, face to face in the presence of water, and then these materials are heated. When these materials are separated from each other after the heating step, a colored image is obtained in the silver halide photosensitive material and the dye is decolorized. In this case, the concentration of the dye after the decolorization is one third or less and preferably one fifth or less of the original concentration. The molar amount of the decolorizing agent to be used is in the range of 0.1 to 200 times and preferably 0.5 to 100 times that of the dye.

In the present invention, a photosensitive material, which comprises a transparent support having thereon at least three photosensitive layers, each layer containing at least photosensitive silver halide grains, a color developing agent, a coupler and a binder wherein the photosensitive wavelength regions differ each other and the absorption wavelength regions of the dyes to be formed from the developing agent and the coupler differ each other, and a processing material, which comprises a support having thereon a processing layer containing at least a base and/or base precursor, are used. These photosensitive material and processing material are placed face to face in such a manner that the photosensitive layer side of the photosensitive material and the processing layer side of the processing material are put together in the presence of water in an amount ranging from  $\frac{1}{10}$  to the equivalent of an amount which is required for the maximum swelling of the total of the layers of the photosensitive material and the processing material except for back layers thereof. These materials are heated, while being put together, for 1 to 120 seconds, preferably for 5 to 60 seconds, in such a manner that the temperature of the faces put together ranges from 50 to 100°C., preferably from 60 to 100°C., to thereby form an image based on the non-diffusive dyes of at least three colors. Furthermore, it is desirable to obtain a color image on other recording material based on the image information obtained in the above-described procedure. Needless to say, the same condition as the above-described condition can be applied to the formation of an image of a single color.

The photosensitive silver halide usable in the present invention (silver halide that contributes to the image formation) may be any of silver iodobromide, silver bromide, silver chlorobromide, silver iodochloride, silver chloride, and silver iodochlorobromide, and mixtures thereof. The grain size of the silver halide is preferably 0.1 to 2  $\mu\text{m}$  and most preferably 0.2 to 1.5  $\mu\text{m}$  based on the diameter of a sphere having an equivalent volume.

The shape of the silver halide grain may be selected from a regularly structured crystal such as a cube, octahedron, or tetradecahedron, and a tabular shape such as a hexagon or rectangle. Among these shapes, preferred is a tabular shape having an aspect ratio of 2 or more, more preferably an aspect ratio of 8 or more, and most preferably an aspect ratio of 20 or more. It is preferable to use an emulsion in which

these tabular grains account for 50% or more, preferably 80% or more, and most preferably 90% or more of the projected area of the total grains.

In addition, preferably used are grains which have a further high aspect ratio and having a thickness less than 0.07  $\mu\text{m}$  as described in U.S. Pat. Nos. 5,494,789; 5,503,970; 5,503,971; 5,536,632 and others.

Furthermore, preferably used are tabular grains which are rich in silver chloride and has (111) face as a main plane as described in U.S. Pat. Nos. 4,400,463; 4,713,323; 5,217,858 and others, and tabular grains which are rich in silver chloride and has (100) face as a main plane as described in U.S. Pat. Nos. 5,264,337; 5,292,632; 5,310,635 and others.

Examples in which these silver halide grains are actually used are described in JP-A Nos. 9-274,295; 9-319,047; 10-115,888 and others.

It is preferable that the silver halide emulsion for the formation of the photosensitive layers in the present invention are normally chemically sensitized and spectrally sensitized.

As for the chemical sensitization, a chalcogen-sensitization method wherein sulfur, selenium or tellurium is used, a noble metal sensitization wherein gold, platinum, iridium or the like is used, a reductive sensitization method wherein a high sensitivity is obtained by introducing reductive silver nuclei using a properly reductive compound during grain formation, and a combination of these methods can be used.

As for the spectral sensitization, so-called spectrally sensitizing dyes, which are adsorbed on silver halide grains and make the grains sensitive to the wavelengths within the region of the absorption wavelengths of the dyes themselves, are used. Examples of these dyes include cyanine dyes, merocyanine dyes, complex cyanine dyes, complex merocyanine dyes, holopolar dyes, hemicyanine dyes, styryl dyes, hemioxonol dyes, and so on. These spectrally sensitizing dyes are used singly or in combinations. It is also preferable to use these dyes in combination with a supersensitizing agent.

In the present invention, it is preferable to add a variety of stabilizers to the silver halide emulsion for photosensitive layers in order to prevent the fogging or to improve the storage stability. Examples of these stabilizers include nitrogen-containing heterocyclic compounds, such as azaindenes, triazoles, tetrazoles and purines, and mercapto compounds such as mercaptotetrazoles, mercaptotriazoles, mercaptoimidazoles and mercaptothiadiazoles.

As for the photographic additives for silver halide emulsions, preferably employed are those described in Journal of Research Disclosure Nos. 17,643 (December, 1978), 18,716 (November, 1979), 307,105 (November, 1989), 38,957 (September, 1996), and others.

The amount to be coated of the silver halide emulsion is generally 0.05 to 20 g/m<sup>2</sup> and preferably 0.1 to 10 g/m<sup>2</sup> based on silver.

The binder of the photosensitive material is preferably a hydrophilic binder. Examples the hydrophilic binders include those described in the above-cited Journal of Research Disclosure and JP-A No. 64-13,546, pages 71-75.

Among these binders, particularly preferred are gelatin and a combination of gelatin with other water-soluble binder such as polyvinyl alcohol, modified polyvinyl alcohol, a cellulose derivative, acrylamide, or the like. The amount to be coated of the binder is generally 1 to 20 g/m<sup>2</sup>, preferably 2 to 15 g/m<sup>2</sup>, and more preferably 3 to 12 g/m<sup>2</sup>. The proportion of gelatin in the binder is generally 50 to 100% and preferably 70 to 100%.

The color developing agent (or precursor thereof) for use in the photosensitive material of the present invention is preferably carbamoyl hydrazine whose structure is described in JP-A No. 8-286,340, p-phenylene diamines, or p-aminophenols. More preferably, the compounds represented by the following general formula (a) or (b) are used as the color developing agent (or precursor thereof).

Examples of the nucleophilic partial structure included in  $Z$  (=indicates non-covalent electron pair and the atom underlined by =has nucleophilicity)



In the general formulae (a) and (b),  $R^{501}$  to  $R^{504}$  each represent a hydrogen atom or a substituent group. Specific examples of the substituent group include the following groups.

A halogen atom (e.g., a chlorine or bromine atom), an alkyl group (e.g., a methyl, ethyl, isopropyl, n-butyl, or t-butyl group), an aryl group (e.g., a phenyl, tolyl, or xylyl group), an carbonamide group (e.g., an acetylamino, propionylamino, butyloylamino, or benzoylamino group), an sulfonamide group (e.g., a methanesulfonylamino, ethanesulfonylamino, benzenesulfonylamino, or toluenesulfonylamino group), an alkoxy group (e.g., a methoxy or ethoxy group), an aryloxy group (e.g., a phenoxy group), an alkylthio group (e.g., a methylthio, ethylthio, or butylthio group), an arylthio group (e.g., a phenylthio or tolylthio group), an carbamoyl group (e.g., a methylcarbamoyl, dimethylcarbamoyl, ethylcarbamoyl, diethylcarbamoyl,

dibutylcarbamoyl, piperidinocarbamoyl, morpholinocarbamoyl, phenylcarbamoyl, methylphenylcarbamoyl ethylphenylcarbamoyl, or benzylphenylcarbamoyl group), a sulfamoyl group (e.g., a methylsulfamoyl, dimethylsulfamoyl, ethylsulfamoyl, diethylsulfamoyl, dibutylsulfamoyl, piperidinosulfamoyl, morpholinosulfamoyl, phenylsulfamoyl, methylphenylsulfamoyl, ethylphenylsulfamoyl, or benzylphenylsulfamoyl), a cyano group, a sulfonyl group (e.g., a methanesulfonyl, ethanesulfonyl, phenylsulfonyl, 4-chlorophenylsulfonyl, or p-toluenesulfonyl group), an alkoxy carbonyl group (e.g., a methoxycarbonyl, ethoxycarbonyl, or butoxycarbonyl group), an aryloxycarbonyl group (e.g., a phenoxy carbonyl group), an acyl group (e.g., an acetyl, propionyl, or butyloyl, benzoyl, or alkylbenzoyl group), a ureido group (e.g., a methylaminocarbonamide or diethylaminocarbonamide group), a urethane group (e.g., a methoxycarbonamide or butoxycarbonamide group), and an acyloxy group (e.g., an acetoxy, propionyloxy, or butyloxy group).

Among  $R^{501}$  to  $R^{504}$ ,  $R^{502}$  and/or  $R^{504}$  are each a hydrogen atom. If  $A^{101}$  is a hydroxyl group, the sum of Hammett constants  $\sigma$  p of  $R^{501}$  to  $R^{504}$  is preferably 0 or more, while if  $A^{101}$  is a substituted amino group, the sum of Hammett constants  $\sigma$  p of  $R^{501}$  to  $R^{504}$  is preferably 0 or less.

$A^{101}$  represents a hydroxyl group or a substituted amino group (e.g., a dimethylamino, diethylamino, or ethylhydroxyethylamino group) and is preferably a hydroxyl group.

In the general formula (a),  $X^{101}$  represents a linking group having a valency of 2 or more and selected from the group consisting of  $-\text{CO}-$ ,  $-\text{SO}-$ ,  $-\text{SO}_2-$ , and  $(\text{Q}^{101})\text{P}(=\text{O})-$  (where  $\text{Q}^{101}$  represents a monovalent substituent group attached to P and specific examples of the substituent group include  $-(\text{Y}_{k1}=\text{Z}_{k1})-\text{D}^{101}$  in addition to the groups listed as the substituent groups of the aforementioned  $R^{501}$  to  $R^{504}$ ; and O is linked to P by way of a double bond).

$\text{Y}_{k1}$  and  $\text{Z}_{k1}$  each represents a nitrogen atom or a group represented by  $-\text{CR}^{505}-$  (where  $\text{R}^{505}$  represents a hydrogen atom or a substituent group). Examples of  $\text{R}^{505}$  include the groups listed as the substituent groups of the aforementioned  $R^{501}$  to  $R^{504}$ .

$k_1$  is an integer of 0 or greater, and is preferably 0, 1 or 3, more preferably 0 or 1, most preferably 0.

$\text{D}^{101}$  represents a proton-dissociative group or a group capable of becoming a cation and having a function to sever the  $\text{N}-\text{X}^{101}$  linkage and to form a dye by the detachment of a substituent group from the coupling position of coupler, triggered by electron transfer from  $\text{D}^{101}$ , after the oxidized product of a compound, which is produced by an oxidation/reduction reaction between a compound represented by the general formula (a) and a silver halide, undergoes a coupling reaction with the coupler. More specifically, after the coupling reaction, electron transfer takes place toward the coupling position from the anion produced by proton dis-

sociation or the non-covalent electron pair of the atom capable of becoming a cation on  $\text{D}^{101}$  to thereby produce a double bond between  $\text{X}^{101}$  and  $\text{Y}_{k1}$  (between  $\text{X}^{101}$  and  $\text{D}^{101}$  when  $k_1$  is 0). As a result, the  $\text{N}-\text{X}^{101}$  linkage is severed and the substituent group on the coupler side is detached as an anion simultaneously with the formation of the double bond between the coupling position on the coupler and the N atom. This series of electron transfer mechanism causes the formation of a dye and detachment of the substituent group. As atoms having the above-mentioned functions, examples of the proton-dissociative atom include an oxygen atom, a sulfur atom, a selenium atom, and a nitrogen or carbon atom substituted by an electron-attractive group or an electron-

rich aromatic group (e.g., an aryl or heteroaromatic group). On the other hand, examples of the atom capable of becoming a cation include a nitrogen atom, a sulfur atom, and so on.

$D^{101}$  is a substituent group containing an atom capable of becoming a trigger for the above-described electron transfer and the atom may be substituted by a variety of substituent groups. The atom may be substituted, for example, by the following groups. An alkyl group (e.g., a methyl, ethyl, isopropyl, n-butyl, or t-butyl group), an aryl group (e.g., a phenyl, tolyl, or xylyl group), an carbonamide group (e.g., an acetylamino, propionylamino, butyloylamino, or benzoylamino group), an sulfonamide group (e.g., a methanesulfonylamino, ethanesulfonylamino, 15 benzenesulfonylamino, or toluenesulfonylamino group), an alkoxy group (e.g., a methoxy or ethoxy group), an aryloxy group (e.g., a phenoxy group), an alkylthio group (e.g., a methylthio, ethylthio, or butylthio group), an arylthio group (e.g., a phenylthio or tolylthio group), an carbamoyl group (e.g., a methylcarbamoyl, dimethylcarbamoyl, ethylcarbamoyl, diethylcarbamoyl, dibutylcarbamoyl, piperidinocarbamoyl, morpholinocarbamoyl, phenylcarbamoyl, methylphenylcarbamoyl, ethylphenylcarbamoyl, or benzylphenylcarbamoyl group), a sulfamoyl group (e.g., a methylsulfamoyl, dimethylsulfamoyl, ethylsulfamoyl, diethylsulfamoyl, dibutylsulfamoyl, 20 piperidinosulfamoyl, morpholinosulfamoyl, phenylsulfamoyl, methylphenylsulfamoyl, ethylphenylsulfamoyl, or benzylphenylsulfamoyl), a cyano group, a sulfonyl group (e.g., a methanesulfonyl, ethanesulfonyl, phenylsulfonyl, 4-chlorophenylsulfonyl, or p-toluenesulfonyl group), an alkoxy carbonyl group (e.g., a methoxycarbonyl, ethoxycarbonyl, or butoxycarbonyl group), an aryloxy carbonyl group (e.g., a phenoxy carbonyl group), an acyl group (e.g., an acetyl, propionyl, or butyloyl, benzoyl, or alkylbenzoyl group), an acyloxy group (e.g., an acetoxy, propionyloxy, or butyloxy group), a ureido group, a urethane group, and a heterocyclic group (e.g., a pyridyl, furyl, or quinolyl group).

Particularly preferred as  $D^{101}$  are an aralkyl group (a benzyl group in particular), an anilino group, a heterocyclic group, a methylene group substituted by an electron-attractive group, and a methine group. These groups may be substituted by a substituent group and examples of the substituent group include a hydroxyl group and the groups listed as the substituent groups of the aforementioned  $R^{501}$  to  $R^{504}$ . Further, at least two atoms or substituent groups selected from  $Y_{k1}$ ,  $Z_{k1}$  and  $D^{101}$  may join together to form a ring.

In the general formula (b),  $X^{201}$  represents a linking group having a valency of 2 or more and selected from the group consisting of  $-\text{CO}-$ ,  $-\text{SO}-$ ,  $-\text{SO}_2-$ , and  $-\text{P}(=\text{O})-$ .

$Z$  represents a nucleophilic group having a function to form a dye by attacking the carbon, sulfur or phosphorus atom of  $X^{201}$ , after the oxidized product of a compound, which is produced as a result of reduction of a silver halide by a compound represented by the general formula (b), undergoes a coupling reaction with a coupler.

What causes nucleophilicity in the nucleophilic group are, as generally observed in the field of organic chemistry, an atom having a non-covalent electron pair (e.g., a nitrogen, phosphorus, oxygen, sulfur, or selenium atom) and an

anionic species (e.g., a nitrogen, oxygen, carbon, or sulfur anion). Examples of the nucleophilic group include the groups having aforementioned partial structures or dissociated forms thereof.

$Y$  represents a divalent linking group. The linking group is a group which links  $Z$  to such a position that conveniently enables the intramolecular nucleophilic attack on  $X^{201}$ . Actually, when the nucleophilic group nucleophilically attacks  $X^{201}$ , the transitional state preferably has atoms linked together such that a 5- or 6-membered ring can be formed.

Preferred examples of  $Y$  include a 1, 2- or 1,3-alkylene group, a 1,2-cycloalkylene group, a  $Z$ -vinylene group, a 1,2-arylene group, a 1,8-naphthylene group, and so on.

$R^{501}$  and  $R^{502}$  may join together to form a ring.  $R^{503}$  and  $R^{504}$  may join together to form a ring. Preferred examples of these rings are 5~6-membered carbon rings or heterocyclic rings.

In the present invention, the compounds represented by the general formula (a) or (b) are preferably oil-soluble compounds. In other word, it is preferable that the compounds represented by the general formula (a) or (2) each have at least one group which has a ballasting property. The term "ballast group" as used herein means a group which imparts the oil-solubility and comprises an oil-soluble partial structure having 8 to 80, preferably 10 to 40, carbon atoms. Because of this, it is preferable that at least one of  $R^{501} \sim R^{502}$ ,  $Y_{k1}$ ,  $Z_{k1}$  and  $D^{101}$  in the general formula (a), and  $X^{201}$ ,  $Y$  and  $Z$  in the general formula (b) has a substituent group having 8 or more carbon atoms.

The color developing agent represented by the general formula (a) or (b) can be added to the silver halide photographic photosensitive material in the following way. First, a coupler, the color developing agent, and an organic solvent having a high boiling point (e.g., an alkyl ester of phosphoric acid, an alkyl ester of phthalic acid, or the like) are mixed together and thereafter dissolved in a solvent having a low boiling point (e.g., ethyl acetate, methyl ethyl ketone, or the like). The solution thus prepared is dispersed in water by an emulsifying method known in the art and the dispersion is added to the photosensitive material. Further, the addition can also be made by the solid dispersion method described in JP-A No. 63-271,339.

The amount to be added of the color developing agent represented by the general formula (a) or (b) has a wide range. But, the amount is preferably 0.01 to 100 times, more preferably 0.1 to 10 times, the molar amount of the coupler.

Although a single color developing agent or a combination of a plurality of color developing agents may be used, the total amount is generally 0.05 to 20 mmol/m<sup>2</sup> and preferably 0.1 to 10 mmol/m<sup>2</sup>.

Specific examples of the compounds (color developing agents D-1 to D-115) represented by the general formula (a) or (b) are given below. It should be understood that the present invention is not limited by these specific examples.



D-1



D-2



D-3



D-4



D-5



D-6



D-7

83

84

-continued

D-8



D-9



D-10



D-11



**85****86**

-continued

D-12



D-13



D-14



D-15



D-16



D-17



D-18



D-19



-continued



D-21

D-20



D-101



D-102



D-104



D-103



D-105

D-106



**89****90**

-continued

D-107



D-108



D-109



D-110



D-111



D-112



D-113



-continued

D-114



D-115

A coupler, which undergoes a coupling reaction with the oxidized product of the color developing agent to form a dye, is used in the photosensitive layer of the photosensitive material. Preferred examples of the coupler include compounds generally called active methylenes, 5-pyrazolones, pyrazoloazoles, phenols, naphthols and pyrrolotriazoles. Specific examples of these couplers are those cited in Journal of Research Disclosure No. 38,957 (June, 1996), pp.616-624. Particularly preferred examples of the coupler include the pyrazoloazole couplers described in JP-A No. 8-110,608, and the pyrrolotriazole couplers described in JP-A Nos. 8-122,994 and 9-218,496. The amount to be used of the coupler is generally 0.05 to 10 mmol/m<sup>2</sup>, preferably 0.1 to 5 mmol/m<sup>2</sup>, for each color.

It is also possible to use a colored coupler, which compensates the unnecessary absorption of coloring dyes, and a compound (including a coupler) which reacts with the oxidized product of the color developing agent to release a photographically useful residue of compound, e.g., a development suppressor.

Normally, the photosensitive material comprises 3 or more photosensitive layers each having a different sensitivity to color. Each photosensitive layer contains at least one-silver halide emulsion layer, and, in a typical example, the photosensitive layer comprises a plurality of silver halide emulsion layers each having substantially the same sensitivity to color but a different photosensitivity. The photosensitive layer is a unit photosensitive layer having sensitivity to any one of blue light, green light and red light. In a multi layered silver halide color photographic photosensitive material, a generally adopted order of the unit photosensitive layers from the support side is a red-sensitive layer, a green-sensitive layer and a blue-sensitive layer. However, depending on the purpose, this order may be reversed, or photosensitive layers sensitive to the same color may sandwich a photosensitive layer sensitive to a different color. The total thickness of the photosensitive layer is generally 1 to 20  $\mu\text{m}$  and preferably 3 to 15  $\mu\text{m}$ .

The silver halide, the color developing agent and the coupler may be incorporated in the same photosensitive layer or in different photosensitive layers. A non-photosensitive layer, such as a protective layer, a primer layer, an intermediate layer, the aforementioned yellow filter layer and antihalation layer, and the like, may be formed in addition to the photosensitive layer. Further, a back layer may be formed on the reverse side of the support. The total thickness of the layers on the photosensitive layer side is generally 3 to 25  $\mu\text{m}$  and preferably 5 to 20  $\mu\text{m}$ .

For various purposes, the photosensitive material may contain such agents as a hardener, a surfactant, a photographic stabilizer, an antistatic agent, a slicking agent, a

matting agent, a latex, a formalin scavenger, a dye, a UV absorber, and so on. Specific examples of these agents are described in the Journal of Research Disclosure cited above, JP-A No. 9-204,031, and others. Particularly preferred examples of the antistatic agent are fine particles of metal oxide such as ZnO, TiO<sub>2</sub>, SnO<sub>2</sub>, Al<sub>2</sub>O<sub>3</sub>,  $\text{In}_2\text{O}_3$ , SiO<sub>2</sub>, MgO, BaO, MoO<sub>3</sub>, V<sub>2</sub>O<sub>5</sub>, and the like.

As for the support of the photosensitive material, preferable are supports for use in photography as described in "Fundamentals of Photographic Engineering—Silver Salt Photography Section", pp.223-240, edited by Photographic Society of Japan, published by Corona Co., Ltd., 1979. Specific examples of the support include polyethylene terephthalate, polyethylene naphthalate, polycarbonate, syndiotactic polystyrene, celluloses (e.g., triacetylcellulose), and so on.

For the purpose of improvement of optical properties and physical properties, these supports may be subjected to a heat treatment (control of degree of crystallization and orientation), uniaxially or biaxially stretching (control of orientation), blending with other polymers, a surface treatment, and so on.

It is preferable to use a support having a magnetic recording layer, described, for example in JP-A Nos. 4,124, 645; 5-40,321; 6-35,092 and 6-31,875, so that the photographing information and others can be recorded.

It is also preferable that the reverse side of the support is coated with a water-proof polymer such as the one described in JP-A No. 8-292,514.

Details of the polyester support, which is particularly preferred for use in the above-described photosensitive material having a magnetic recording layer, are described in Journal of Technical Disclosure No. 94-6023 (issued on Mar. 15, 1994 from The Japan Institution of Innovation and Invention).

The thickness of the support is generally 5 to 200  $\mu\text{m}$  and preferably 40 to 120  $\mu\text{m}$ .

The combination, as a base precursor, of a basic metal compound poorly soluble in water and a compound which can cause a complex forming reaction with the metal ion constituting the metal compound (referred to as complex forming compound) is described in JP-A No. 62-12,848, European Patent Application Laid-Open No. 210,660A2, U.S. Pat. No. 4,740,445, and others.

The basic metal compounds, poorly soluble in water, for use in the photosensitive material are oxides, hydroxides, and basic carbonates of zinc or aluminum, and most preferably zinc oxide, zinc hydroxide, and zinc basic carbonate.

The basic metal compounds poorly soluble in water is utilized as a dispersion of fine particles in a hydrophilic binder as described in JP-A No. 59-174,830. The average

particle diameter of the fine particles is 0.001 to 5  $\mu\text{m}$  and preferably 0.01 to 2  $\mu\text{m}$ . The content of the basic metal compound in the photosensitive material is 0.01 to 5 g/m<sup>2</sup> and preferably 0.05 to 2 g/m<sup>2</sup>.

The complex forming compound to be used in the processing material is a compound known as a chelating agent in analytical chemistry and a compound known as a softener for hard water in photographic chemistry. Details of the complex forming compound are described in the official gazettes cited above and also in A. Ringbom, "Complex Forming Reaction", translated by N. Tanaka and H. Sugi (sangyo Tosho Publishing Co., Ltd.). The complex forming compound preferable as the one for use in the present invention is a water-soluble compound. Example of the compound include an aminopolycarboxylic acid (including salt thereof) such as ethylenediaminetetraacetic acid, nitrilotriacetic acid, diethylenetriaminepentaacetic acid or the like, an aminophosphonic acid (salt) such as aminotris (methyleneephosphonic acid), ethylenediaminetetramethyleneephosphonic acid or the like, pyridinecarboxylic acid (salt) such as 2-picolinic acid, pyridine-2,6-dicarboxylic acid, 5-ethyl-2-picolinic acid or the like. Among these compounds, the pyridinecarboxylic acid (salt) is particularly preferable.

In the present invention, it is preferable that the complex forming compound is used as a salt produced by neutralization with a base. In particular, preferred examples are salts with organic bases such as guanidines, amidines, hydroxytetraalkylammoniums, and the like, and salts with alkaline metals such as sodium, potassium, lithium and the like as well as mixtures of these salts. Specific examples of these preferred complex forming compounds are described in above-cited JP-A No. 129,848, European Patent Application Laid-Open No. 210,660A2, and others. The content of the complex forming compound in the processing material is 0.01 to 10 g/m<sup>2</sup> and preferably 0.05 to 5 g/m<sup>2</sup>.

The processing material may contain a mordant and the mordant is preferably a polymeric one.

As described in JP-A No. 9-146,246, the processing material may contain physical development nuclei such as colloidal silver or palladium sulfide and a solvent for silver halide such as hydantoin so that the silver halide in the photosensitive material is solubilized simultaneously with development and fixed to the processing material.

Further, the processing material may contain a development stopper, a printout preventing agent, and so on.

The processing material may have a protective layer, a primer layer, a back layer, and other auxiliary layers besides the processing layer.

The processing material is preferably composed of a continuous web and a processing layer coated thereon in order that part of the processing material, after being fed from delivery rolls and used in processing, does not need to be cut and is wound on other roll. This example is described in JP-A No. 9-127,670.

The support for the processing material is not particularly limited and plastic films or paper, such as those listed in the explanation of the photosensitive material, may be used. The thickness is 4 to 120  $\mu\text{m}$  and preferably 6 to 70  $\mu\text{m}$ .

The film which is vacuum-deposited with aluminum and is described in JP-A No. 9-222,690 can be preferably used.

One of the methods for supplying water at the time of heat development is a method wherein a photosensitive material or processing material is immersed in water and thereafter the excess water is removed by means of a squeezing roller. Other preferred method is described, for example, in JP-A No. 10-26,817. This method uses a water spraying apparatus

comprising a plurality of nozzles which eject water and are linearly arranged at certain intervals in the direction perpendicular to the direction of the transfer of the photosensitive material or processing material and also actuators which displace the nozzles in the direction of the photosensitive material or processing material being transferred. Further, a method wherein water is coated with of a sponge or the like onto the photosensitive material or processing material is also suitable.

Examples of the heating method in the developing process include a method in which the materials are brought into contact with a heated block or plate, and a method which employs a heat roller, a heat drum, or an infrared or far infrared lamp.

In the present invention, a separate bleaching/fixing step, intended for the removal of the silver halide remaining in the photosensitive material after development or for further removal of the developed silver, is not essential. However, a fixing step and/or a bleaching step may be employed in order to lessen the load on reading image information and to enhance the storage stability of images. If these steps employed, although these steps may be carried out by ordinary treatments using liquids, it is preferable to employ a step in which the photosensitive material is heated after being put together with other sheet coated with a processing agent as described in JP-A No. 9-258,402.

According to the present invention, after an image is obtained on the photosensitive material, it is preferable to use the image to obtain a color image on other recording material. Although this process may be performed by an ordinary projection exposure using a photosensitive material such as color paper, a preferred method for this purpose comprises the steps of photoelectrically reading the image information by measuring the intensity of the transmitted light, converting the data into digital signals, and outputting the signals onto other recording material after image treatment. The material on which the output is made may be a sublimation-type heat sensitive recording material, a full-color direct heat-sensitive recording material, an ink-jet material, an electro-photographing material, or the like in addition to a photosensitive material using silver halide.

Besides, the photosensitive material of the present invention can also be developed by a liquid-based developing method for ordinary photosensitive materials described in Journal of Research Disclosures No. 17,642, pp.28-29, No. 18,716, pp.651, left to right column, and No. 307,105, pp.880-881, each cited previously.

## EXAMPLES

In order to better explain the present invention, the following examples are given by way of illustration and not by way of limitation. In the following examples and comparative examples, "%" means "weight %" unless otherwise specified.

### Preparation of Photosensitive Emulsion

A mixture of 0.74 g of gelatin having an average molecular weight of 15,000, 0.7 g of potassium bromide, and 930 mL of distilled water was placed in a reaction vessel, and thereafter the temperature of the mixture was raised to 40° C. To this solution, which was vigorously stirred, there were added 30 mL of an aqueous solution containing 0.34 g of silver nitrate and 30 mL of an aqueous solution containing 0.24 g of potassium bromide over a period of 20 seconds. Upon completion of the addition, after the reaction solution was kept at 40° C. for 1 minute, the temperature was raised to 75° C.

Next, 27.0 g of gelatin and 200 mL of distilled water were added together to the reaction solution. After that, 100 mL of an aqueous solution containing 23.26 g of silver nitrate and 80 mL of an aqueous solution containing 16.37 g of potassium bromide were added to the reaction solution over a period of 36 minutes in such a manner that the flow rate of the addition was gradually increased. Further, 250 mL of an aqueous solution containing 83.2 g of silver nitrate and an aqueous solution containing potassium iodide and potassium bromide at a molar ratio of the former to the latter of 3:97 (having a potassium bromide concentration of 26%) were added to the reaction solution over a period of 60 minutes in such a manner that the flow rate of the addition was gradually increased and that the silver potential of the reaction solution was -20 mV with reference to a saturated calomel electrode. Furthermore, 75 mL of an aqueous solution containing 18.7 g of silver nitrate and a 21.9% potassium bromide aqueous solution were added to the reaction solution over a period of 10 minutes in such a manner that the silver potential of the reaction solution was 20 mV with reference to a saturated calomel electrode. After the completion of the addition, the temperature of the reaction solution was kept at 75° C. for 1 minute, and the temperature of the reaction solution was then lowered to 40° C. Then, 100 mL of an aqueous solution containing 10.5 g of sodium p-iodoacetamidebenzenesulfonate monohydrate to adjust the pH of the reaction solution to 9.0. Further, 50 mL of an aqueous solution containing 4.3 g of sodium sulfite was added. After the addition, the reaction solution was kept at 40° C. for 3 minutes, and the temperature of the reaction solution was then raised to 55° C. Next, after the pH of the reaction solution was adjusted to 5.8, 0.8 mg of sodium benzenethiosulfinate, 0.04 mg of potassium hexachloroiridate (IV) and 5.5 g of potassium bromide were added to the reaction solution. After the completion of the addition, the temperature of the reaction solution was kept at 55° C. for 1 minute. Then, 180 mL of an aqueous solution containing 44.3 g of silver nitrate and 160 mL of an aqueous solution containing 34.0 g of potassium bromide and 8.9 mg of potassium hexacyanoferrate (II) were added to the reaction solution over a period of 30 minutes. The temperature of the reaction solution was then lowered, and a desalting treatment was performed by a standard method. After the desalting treatment, gelatin was added to the reaction solution such that the gelatin content became 7% by weight and the pH of the reaction solution was adjusted to 6.2.

The emulsion obtained was made up of hexagonal tabular grains having an average grain size expressed in an equivalent-sphere diameter of  $1.29 \mu\text{m}$ , an average grain thickness of  $0.27 \mu\text{m}$  and having an average aspect ratio, i.e., a ratio obtained by dividing the projected grain diameter by grain thickness, of 8.5. This emulsion was designated as emulsion A-1.

The procedure of the preparation of Emulsion A-1 was repeated, except that the amounts of the silver nitrate and potassium bromide to be added at the initial stage of grain formation were changed so as to change the number of nuclei to be formed. The emulsion obtained in this way was made up of hexagonal tabular grains having an average grain size expressed in an equivalent-sphere diameter of  $0.75 \mu\text{m}$ , an average grain thickness of  $0.18 \mu\text{m}$  and an average aspect ratio of 6.9. This emulsion was designated as emulsion A-2. Further, the procedure of the preparation of Emulsion A-1 was repeated, except that the amounts of the silver nitrate and potassium bromide to be added at the initial stage of grain formation were changed. The emulsion obtained in this way was made up of hexagonal tabular grains having an

average grain size expressed in an equivalent-sphere diameter of  $0.52 \mu\text{m}$ , an average grain thickness of  $0.18 \mu\text{m}$  and an average aspect ratio of 4.0. This emulsion was designated as emulsion A-3. In these preparations, the amounts of the potassium hexachloroiridate (IV) and potassium hexacyanoferrate (II) were changed in inverse proportion to the grain volume while the amount of the sodium p-iodoacetamidebenzenesulfonate monohydrate was changed in proportion to the length of grain periphery.

10 Next, 5.6 mL of 1% aqueous solution of potassium iodide was added to Emulsion A-1 at 40° C. After the addition, the spectral sensitization and the chemical sensitization of this emulsion were performed by the addition thereto of the following blue-sensitizing dye in an amount of  $6.1 \times 10^{-4}$  mol/mol of silver, the following compound I as a stabilizer in an amount of  $1 \times 10^{-5}$  mol/mol of silver, potassium thiocyanate, chloroauric acid, sodium thiosulfate and mono (pentafluorophenyl)diphenylphosphine selenide as chemical sensitizers. After the completion of the spectral sensitization and chemical sensitization, the following stabilizer S was added. The amounts of the chemical sensitizers were adjusted so that the level of the chemical sensitization of the emulsion was optimized.

## Blue-sensitizing Dye



### Compound I (Stabilizer)



#### Stabilizer S (Mixture of the Following Compounds)



60  $2 \times 10^{-4}$  mol/molAg of silver  $8 \times 10^{-5}$  mol/molAg for the emulsion A-1

The blue-sensitive emulsion thus prepared was designated as A-1 b. Similarly, the spectral sensitization and chemical sensitization for the emulsions A-2 and A-3 were conducted so as to prepare blue-sensitive emulsion A-2 b and blue-sensitive emulsion A-3 b, except that the amounts of the spectral sensitizing dyes were changed in accordance with

97

the surface area of the silver halide grains in the emulsions. On the other hand, the amounts of the chemical sensitizers were adjusted so that the levels of the chemical sensitization of the emulsions were optimized.

Furthermore, green-sensitive emulsions A-1 g, A-2 g and A-3 g were prepared by replacing the bleu-sensitizing dyes by the following green-sensitizing dyes I to III, while red-sensitive emulsions A-1 r, A-2 r and A-3 r were prepared by replacing the bleu-sensitizing dyes by the following red-sensitizing dyes I to III.

Green-sensitizing Dye I



5.5×10<sup>-4</sup> mol/mol of silver for the emulsion A-1

Green-sensitizing Dye II



1.3×10<sup>-4</sup> mol/mol of silver for the emulsion A-1

Green-sensitizing Dye III



4.8×10<sup>-5</sup> mol/mol of silver for the emulsion A-1

Red-sensitizing Dye I



2.5×10<sup>-4</sup> mol/mol of silver for the emulsion A-1

98

Red-sensitizing Dye II



6.3×10<sup>-5</sup> mol/mol of silver for the emulsion A-1  
Red-sensitizing Dye III



25 3×10<sup>-4</sup> mol/mol of silver for the emulsion A-1

Preparation of a Dispersion of Zinc Hydroxide

30 Next, a dispersion of zinc hydroxide serving as a base precursor was prepared in the following way.

A mixture, which comprised 31 g of zinc hydroxide powder having an average diameter of primary particles of 0.2  $\mu$ m, 1.6 g of carboxymethylcellulose and 0.4 g of sodium 35 polyacrylate as dispersants, 8.5 g of lime-treated ossein gelatin and 158.5 mL of water, was dispersed for one hour by means of a mill with glass beads. After filtering off the glass beads from the mixture, 188 g of a dispersion of zinc hydroxide was obtained.

40 Preparation of an Emulsified Dispersion Liquid Containing a Coupler and an Incorporated Color Developing Agent

45 An emulsified dispersion liquid containing a coupler and an incorporated color developing agent (hereinafter referred to simply as "developing agent" upon occasion) was prepared in the following way.

50 Emulsified Dispersion Liquid Containing a Yellow Coupler and a Developing Agent

A mixture, which comprised 8.95 g of the following 55 yellow coupler (a), 7.26 g of the following developing agent (b), 1.47 g of the following developing agent (c), 0.17 g of the following anti-fogging agent (d), 0.28 g of the following anti-fogging agent (e), 18.29 g of the following organic solvent having a high boiling point (f) and 50.0 mL of ethyl acetate, was made into a solution at 60° C. The solution was 60 blended into 200 g of an aqueous solution comprising 18.0 g of a lime-treated gelatin and 0.8 g of sodium dodecylbenzenesulfonate. The resultant mixture was emulsified by means of a dissolver-type mixing device rotating at 10,000 revolutions per minute over a period of 20 minutes. After the 65 emulsification, distilled water was added to the emulsion so that the total volume became 300 g, and the resultant emulsion was mixed at 2,000 revolutions per minute for 10

99

minutes. In this way, an emulsified dispersion liquid containing a yellow coupler and a developing agent was obtained.



#### Emulsified Dispersion Liquid Containing a Magenta Coupler and a Developing Agent

A mixture, which comprised 7.65 g of the following magenta coupler (g), 1.12 g of the following magenta coupler (h), 8.13 g of the following developing agent (i), 1.05 g of the above-mentioned developing agent (c), 0.11 g of the above-mentioned anti-fogging agent (d), 7.52 g of the following organic solvent having a high boiling point (i) and 38.0 mL of ethyl acetate, was made into a solution at 60° C.

100

The solution was blended into 150 g of an aqueous solution comprising 12.2 g of a lime-treated gelatin and 0.8g of sodium dodecylbenzenesulfonate. The resultant mixture was emulsified by means of a dissolver-type mixing device rotating at 10,000 revolutions per minute over a period of 20 minutes. After the emulsification, distilled water was added to the emulsion so that the total volume became 300 g, and the resultant emulsion was mixed at 2,000 revolutions per minute for 10 minutes. In this way, an emulsified dispersion liquid containing a magenta coupler and a developing agent was obtained.

#### Emulsified Dispersion Liquid Containing a Cyan Coupler and a Developing Agent

A mixture, which comprised 10.78 g of the following cyan coupler (k), 8.23 g of the following magenta coupler (i), 1.06 g of the above-mentioned developing agent (c), 0.15 g of the above-mentioned anti-fogging agent (d), 8.27 g of the following organic solvent having a high boiling point (j) and 38.0 mL of ethyl acetate, was made into a solution at 60° C. The solution was blended into 150 g of an aqueous solution comprising 12.2 g of a lime-treated gelatin and 0.8 g of sodium dodecylbenzenesulfonate. The resultant mixture was emulsified by means of a dissolver-type mixing device rotating at 10,000 revolutions per minute over a period of 20 minutes. After the emulsification, distilled water was added to the emulsion so that the total volume became 300 g, and the resultant emulsion was mixed at 2,000 revolutions per minute for 10 minutes. In this way, an emulsified dispersion liquid containing a cyan coupler and a developing agent was obtained.

Magenta coupler (g)



101  
-continued

Developing agent (i)



Cyan coupler (k)



## Example 1 to 13

## Preparation of Support

A support used in Example 1 was prepared as follows.

100 parts by weight of a polyethylene-2,6-naphthalate (PEN) polymer and 2 parts by weight of Tinuvin P.326 (manufactured by Ciba-Geigy Co.) as an ultraviolet absorber were dried, melted at 300° C., and extruded from a T-die. The resultant material was longitudinally stretched by 3.3 times at 140° C., then transversely stretched by 3.3 times at 130° C., and thermally fixed at 250° C. for 6 seconds. The result was a 90  $\mu\text{m}$ -thick PEN film. Proper amounts of blue, magenta and yellow dyes (I-1, I-4, I-6, I-24, I-26, I-27 and II-5 described in Journal of Technical Disclosure No.94-6, 023) were added to this PEN film so that a yellow density of 0.01, a magenta density of 0.08 and a cyan density of 0.09 were obtained. The PEN film was wound around a stainless steel core having a diameter of 20 cm and given a thermal hysteresis of 30 hours at 113° C., thereby manufacturing a support with a high resistance to curling.

## Formation of Primer Layers

The two surfaces of the support were subjected to corona discharge, UV irradiation and glow discharge and thereafter coated, by using a bar coater, each with 10 cc/m<sup>2</sup> of a primer solution consisting of gelatin (0.1 g/m<sup>2</sup>), sodium  $\alpha$ -sulfo-di-2-ethylhexylsuccinate (0.01 g/m<sup>2</sup>), salicylic acid (0.025 g/m<sup>2</sup>), the following PQ-1 (0.005 g/m<sup>2</sup>), and the following PQ-2 (0.006 g/m<sup>2</sup>). Drying was performed at 115° C. for 6 minutes (all of the rollers and conveyors in the drying zone were maintained at 115° C.).

## 102

## Formation of Back Layer

## (1) Formation of Antistatic Layer

5 The support was coated with a mixture composed of a dispersion (secondary aggregate particle size: about 0.08  $\mu\text{m}$  (0.027 g/m<sup>2</sup>) of a fine powder of a tin oxide/antimony oxide composite material having an average particle size of 0.005  $\mu\text{m}$  and a specific resistance of 5 $\Omega\text{-cm}$ , gelatin (0.03 g/m<sup>2</sup>), (CH<sub>2</sub>=CHSO<sub>2</sub>CH<sub>2</sub>CH<sub>2</sub>NHCO)<sub>2</sub>CH<sub>2</sub> (0.02 g/m<sup>2</sup>), polyoxyethylene-p-nonylphenol (polymerization degree: 10) (0.005 g/m<sup>2</sup>), the following PQ-3 (0.008 g/m<sup>2</sup>), and resorcin (0.001 g/m<sup>2</sup>)

15 (2) Formation of Magnetic Recording Layer  
0.006 g/m<sup>2</sup> of cobalt- $\gamma$ -iron oxide (specific surface area: 43 m<sup>2</sup>/g; major axis: 0.14  $\mu\text{m}$ ; minor axis: 0.03  $\mu\text{m}$ ; saturation 20 magnetization: 89 emu/g; Fe<sup>+2</sup>/Fe<sup>+3</sup>:6/94; surface-treated with aluminum oxide/silicon oxide in an amount corresponding to 2% by weight of the iron oxide) coated with 3-polyoxyethylene-propoxytrimethoxysilane (polymerization degree: 15) (15% by weight), 1.15 g/m<sup>2</sup> of 25 diacetylcellulose (iron oxide was dispersed by means of an open kneader and a sand mill), and the following PQ-4 (0.075 g/m<sup>2</sup>) and the following PQ-5 (0.004 g/m<sup>2</sup>), as hardeners, were applied by means of a bar coater by using 30 acetone, methyl ethyl ketone, cyclohexanone, and dibutyl phthalate as solvents, thus forming a 1.2  $\mu\text{m}$ -thick magnetic layer. Further, 5 mg/m<sup>2</sup> of C<sub>6</sub>H<sub>13</sub>CH(OH) C<sub>10</sub>H<sub>20</sub>COOC<sub>40</sub>H<sub>81</sub> (50 mg/m<sup>2</sup>) as a slicking agent, 15 mg/m<sup>2</sup> of silica particles (average particle diameter: 0.1  $\mu\text{m}$ ) 35 as a matting agent, and 15 mg/m<sup>2</sup> of aluminum oxide particles (ERC-DBM; average particle diameter: 0.44  $\mu\text{m}$ , manufactured by Reynolds Metal Corporation) as an abrasive, were added. Drying was performed at 115° C. for 40 6 minutes (all of the rollers and conveyors in the drying zone were maintained at 115° C.). The color density increment of DB of the magnetic recording layer as measured by an X-light (blue filter) was 0.1. The saturation magnetization moment, coercive force, and squareness ratio of the magnetic recording layer were 4.2 emu/g, 7.5 $\times$ 10<sup>4</sup> A/m, and 45 65%, respectively.

## (3) Formation of Sliding Layer

A mixture of hydroxyethylcellulose (25 mg/m<sup>2</sup>), the following PQ-6 (7.5 g/m<sup>2</sup>), the following PQ-7 (1.5 g/m<sup>2</sup>), and a polydimethylsiloxane (1.5 mg/m<sup>2</sup>) was applied. It should be noted that this mixture was melted in xylene/propyleneglycolmonomethyl ether (1/1) at 105° C., added to and dispersed in propyleneglycolmonomethyl ether (tenfold amount) at room temperature, and formed into a dispersion (average particle size: 0.01  $\mu\text{m}$ ) in acetone before being added. Drying was performed at 115° C. for 6 minutes (all of the rollers and conveyors in the drying zone were maintained at 115° C.) The resultant sliding layer was found to have excellent characteristics. That is, the coefficient of kinetic friction was 0.10 (stainless steel hard ball having a diameter of 5 mm; load: 100 g; speed: 6 cm/minute) and the coefficient of static friction was 0.09 (clip method). The coefficient of kinetic friction between an emulsion surface described previously and the sliding layer was also excellent and gave a value of 0.18.



30

## Dye for Magenta Filter Layer

(CH<sub>3</sub>O)<sub>3</sub>SiCH<sub>2</sub>CH<sub>2</sub>CH<sub>2</sub>O(CH<sub>2</sub>CH<sub>2</sub>O)<sub>n</sub>CH<sub>3</sub> (n=7.3)(C<sub>50</sub>H<sub>101</sub>(CH<sub>2</sub>CH<sub>2</sub>O)<sub>n</sub>H (n=16)

Preparation of Dye Compositions for Yellow Filter  
Layer, Magenta Filter Layer, and Antihalation  
Layer

The dye compositions (decolorizing dye compositions) for yellow filter layer, magenta filter layer, and antihalation layer were prepared as follows.

## Dye for Yellow Filter Layer

The dye for yellow filter layer was prepared as an emulsified dispersion.

7.1 g of the following yellow dye (1) was dissolved in a mixture of 7.1 g of the following organic solvent having a high boiling point (m), 30 mL of ethyl acetate and 30 mL of cyclohexanone. The solution was blended into 135 g of a 7.8% aqueous solution of gelatin containing 1.25 g of sodium dodecylbenzenesulfonate. The resultant mixture was emulsified by means of a dissolver-type mixing device rotating at 10,000 revolutions per minute over a period of 20 minutes. After the emulsification, distilled water was added to the emulsion so that the total volume became 260 g, and the resultant emulsion was mixed at 2,000 revolutions per minute for 10 minutes. In this way, an emulsified dispersion of dye for yellow filter layer was prepared.

PQ-5

The dye for magenta filter layer was also prepared as an emulsified dispersion.

PQ-6

6.1 g of the following yellow dye (n) was dissolved in a mixture of 6.1 g of the following organic solvent having a high boiling point (o), 30 mL of ethyl acetate and 30 mL of cyclohexanone. The solution was blended into 135 g of a 7.8% aqueous solution of gelatin containing 0.46 g of sodium dodecylbenzenesulfonate. The resultant mixture was emulsified by means of a dissolver-type mixing device rotating at 10,000 revolutions per minute over a period of 20 minutes. After the emulsification, distilled water was added to the emulsion so that the total volume became 260 g, and the resultant emulsion was mixed at 2,000 revolutions per minute for 10 minutes. In this way, an emulsified dispersion of dye for magenta filter layer was prepared.

PQ-7

40

45

50

## Dye for Antihalation Layer

The dye (cyan dye) for antihalation layer was prepared as a dispersion of solid fine particles.

2.64 g of a 10 weight % aqueous solution of the following surfactant (p) and 94 mL of water were added to 3.0 g of the cyan dye as the illustrative compound (F-81). The mixture was dispersed by means of a sand grinder mill with zirconia beads having an average diameter of 0.5 mm for 24 hours. After the dispersing operation, the beads were separated and the dye for antihalation layer was prepared as a dispersion of solid fine particles. The particle size of the dispersion of solid fine particles was measured by Master Sizer, manufactured by Malvern Corporation, and the average particle diameter was found to be 0.16  $\mu\text{m}$ .

Yellow dye (1)



A 1:1 mixture of organic solvent having a high boiling point (m) and EMPARA K65 (manufactured by Ajinomoto Co., Ltd.)



Organic solvent having a high boiling point (o)



By using the above-described support and materials, the multi layered photosensitive material 101 shown in the following Tables 1 to 3 was prepared.

TABLE 1

TABLE 1-continued

| 5  | Coating weight of each compound in mg/m <sup>2</sup> constituting photosensitive material 101 |
|----|-----------------------------------------------------------------------------------------------|
|    | Water-soluble polymer (s) 15                                                                  |
|    | Yellow-coloring layer (high-sensitive layer)                                                  |
| 10 | Lime-treated gelatin 1750                                                                     |
|    | Emulsion A-1b                                                                                 |
|    | (based on the coating amount of silver) 635                                                   |
|    | Yellow coupler (a) 298                                                                        |
|    | Developing agent (b) 242                                                                      |
|    | Developing agent (c) 50                                                                       |
| 15 | Anti-fogging agent (d) 5.8                                                                    |
|    | Anti-fogging agent (e) 9.5                                                                    |
|    | Organic solvent having a high boiling point (f) 500                                           |
|    | Surfactant (y) 27                                                                             |
|    | Water-soluble polymer (s) 1                                                                   |
| 20 | Yellow-coloring layer (medium-sensitive layer)                                                |
|    | Lime-treated gelatin 1400                                                                     |
|    | Emulsion A-2b                                                                                 |
|    | (based on the coating amount of silver) 280                                                   |
|    | Yellow coupler (a) 277                                                                        |
| 25 | Developing agent (b) 225                                                                      |
|    | Developing agent (c) 46                                                                       |
|    | Anti-fogging agent (d) 5.3                                                                    |
|    | Anti-fogging agent (e) 8.8                                                                    |
|    | Organic solvent having a high boiling point (f) 566                                           |
| 30 | Surfactant (y) 25                                                                             |
|    | Water-soluble polymer (s) 2                                                                   |
|    | Yellow-coloring layer (low-sensitive layer)                                                   |
|    | Lime-treated gelatin 1400                                                                     |
| 35 | Emulsion A-3b                                                                                 |
|    | (based on the coating amount of silver) 285                                                   |
|    | Yellow coupler (a) 277                                                                        |
|    | Developing agent (b) 225                                                                      |
|    | Developing agent (c) 46                                                                       |
|    | Anti-fogging agent (d) 5.3                                                                    |
| 40 | Anti-fogging agent (e) 8.8                                                                    |
|    | Organic solvent having a high boiling point (f) 566                                           |
|    | Surfactant (y) 25                                                                             |
|    | Water-soluble polymer (s) 2                                                                   |

TABLE 2

|                                                     |                                                          |
|-----------------------------------------------------|----------------------------------------------------------|
| <u>Intermediate layer<br/>(yellow filter layer)</u> |                                                          |
| 50                                                  | Lime-treated gelatin 560                                 |
|                                                     | Surfactant (y) 15                                        |
|                                                     | Surfactant (r) 24                                        |
|                                                     | Yellow dye (l) 85                                        |
|                                                     | Organic solvent having a high boiling point (m) 85       |
| 55                                                  | Zinc hydroxide 125                                       |
|                                                     | Water-soluble polymer (s) 15                             |
|                                                     | <u>Magenta-coloring layer<br/>(high-sensitive layer)</u> |
| 60                                                  | Lime-treated gelatin 781                                 |
|                                                     | Emulsion A-1g                                            |
|                                                     | (based on the coating amount of silver) 1635             |
|                                                     | Magenta coupler (g) 80                                   |
|                                                     | Magenta coupler (h) 12                                   |
|                                                     | Developing agent (i) 85                                  |
|                                                     | Developing agent (c) 11                                  |
|                                                     | Anti-fogging agent (d) 1.2                               |
| 65                                                  | Organic solvent having a high boiling point (j) 79       |
|                                                     | Surfactant (y) 8                                         |

TABLE 2-continued

|                                                    |      |
|----------------------------------------------------|------|
| Water-soluble polymer (s)                          | 8    |
| Magenta-coloring layer<br>(medium-sensitive layer) |      |
| Lime-treated gelatin                               | 659  |
| Emulsion                                           | A-2g |
| (based on the coating amount of silver)            | 935  |
| Magenta coupler (g)                                | 103  |
| Magenta coupler (h)                                | 15   |
| Developing agent (i)                               | 110  |
| Developing agent (c)                               | 14   |
| Anti-fogging agent (d)                             | 1.5  |
| Organic solvent having a high boiling point (j)    | 102  |
| Surfactant (y)                                     | 11   |
| Water-soluble polymer (s)                          | 14   |
| Magenta-coloring layer<br>(low-sensitive layer)    |      |
| Lime-treated gelatin                               | 711  |
| Emulsion                                           | A-3g |
| (based on the coating amount of silver)            | 550  |
| Magenta coupler (g)                                | 274  |
| Magenta coupler (h)                                | 40   |
| Developing agent (i)                               | 291  |
| Developing agent (c)                               | 38   |
| Anti-fogging agent (d)                             | 3.9  |
| Organic solvent having a high boiling point (j)    | 269  |
| Surfactant (y)                                     | 29   |
| Water-soluble polymer (s)                          | 14   |

TABLE 3

Intermediate layer  
(magenta filter layer)

Lime-treated gelatin  
Surfactant (y)  
Surfactant (r)  
Magenta dye (n)  
Organic solvent having a high boiling point (o)  
Formalin scavenger (u)  
Zinc hydroxide  
Water-soluble polymer (s)  
Cyan-coloring layer  
(high-sensitive layer)

Lime-treated gelatin  
Emulsion  
(based on the coating amount of silver)  
Cyan coupler (k)  
Developing agent (i)  
Developing agent (c)  
Anti-fogging agent (d)  
Organic solvent having a high boiling point (j)  
Surfactant (y)  
Water-soluble polymer (s)  
Cyan-coloring layer  
(medium-sensitive layer)

|                                                     |      |
|-----------------------------------------------------|------|
| Lime-treated gelatin                                | 475  |
| Emulsion                                            | A-2r |
| (based on the coating amount of silver)             | 1135 |
| Cyan coupler (k)                                    | 134  |
| Developing agent (i)                                | 102  |
| Developing agent (c)                                | 13   |
| Anti-fogging agent (d)                              | 1.9  |
| Organic solvent having a high boiling point (j)     | 103  |
| Surfactant (y)                                      | 10   |
| Water-soluble polymer (s)                           | 15   |
| Cyan-coloring layer<br><u>(low-sensitive layer)</u> |      |
| Lime-treated gelatin                                | 825  |
| Emulsion                                            | A-3r |
| (based on the coating amount of silver)             | 720  |
| Cyan coupler (k)                                    | 234  |

TABLE 3-continued

|                                                    |     |
|----------------------------------------------------|-----|
| Developing agent (i)                               | 179 |
| Developing agent (c)                               | 23  |
| Anti-fogging agent (d)                             | 3.3 |
| Organic solvent having a high boiling point (j)    | 179 |
| Surfactant (y)                                     | 17  |
| Water-soluble polymer (s)                          | 10  |
| <u>Antihalation layer</u>                          |     |
| 10 Lime-treated gelatin                            | 440 |
| Dye (illustrative compound F-81)                   | 132 |
| Surfactant (p)                                     | 12  |
| Water-soluble polymer (s)                          | 15  |
| Primer layer                                       |     |
| PEN support having a thickness of 92 $\mu\text{m}$ |     |
| 15 Primer layer                                    |     |
| Antistatic layer                                   |     |
| Magnetic recording layer                           |     |
| Sliding layer                                      |     |

20 Further, processing materials P-1 and P-2 as shown in Tables 4 and 5 were prepared.

TABLE 4

## Construction of processing material P-1

|    | Layer construction                          | Materials added                                  | Amounts added (mg/m <sup>2</sup> ) |
|----|---------------------------------------------|--------------------------------------------------|------------------------------------|
| 30 | 4 <sup>th</sup> layer protective layer      | Acid-treated gelatin                             | 220                                |
|    |                                             | Water-soluble polymer (v)                        | 60                                 |
|    |                                             | Water-soluble polymer (W)                        | 200                                |
|    |                                             | Additive (x)                                     | 80                                 |
|    |                                             | Potassium nitrate                                | 16                                 |
|    |                                             | Matting agent (z)                                | 10                                 |
| 35 | 3 <sup>rd</sup> layer intermediate layer    | Surfactant (r)                                   | 7                                  |
|    |                                             | Surfactant (aa)                                  | 7                                  |
|    |                                             | Surfactant (ab)                                  | 10                                 |
|    |                                             | Lime-treated gelatin                             | 240                                |
|    |                                             | Water-soluble polymer (W)                        | 24                                 |
|    |                                             | Hardener (ac)                                    | 180                                |
| 40 | 2 <sup>nd</sup> layer base generating layer | Surfactant (y)                                   | 9                                  |
|    |                                             | Lime-treated gelatin                             | 2100                               |
|    |                                             | Water-soluble polymer (W)                        | 360                                |
|    |                                             | Water-soluble polymer (ad)                       | 700                                |
|    |                                             | Water-soluble polymer (ae)                       | 600                                |
|    |                                             | Organic solvent having a high boiling point (af) | 2120                               |
| 45 | 1 <sup>st</sup> layer primer layer          | Additive (ag)                                    | 20                                 |
|    |                                             | Guanidine picolinate                             | 2613                               |
|    |                                             | Potassium quinolinate                            | 225                                |
|    |                                             | Sodium quinolinate                               | 192                                |
|    |                                             | Surfactant (y)                                   | 24                                 |
|    |                                             | Lime-treated gelatin                             | 247                                |
| 50 | Transparent support (63 µm)                 | Water-soluble polymer (v)                        | 12                                 |
|    |                                             | Surfactant (r)                                   | 14                                 |
|    |                                             | Hardener (ac)                                    | 178                                |

TABLE 5

## Construction of processing material P-2

|    | Layer construction                       | Materials added                                           | Amounts added (mg/m <sup>2</sup> ) |
|----|------------------------------------------|-----------------------------------------------------------|------------------------------------|
| 60 | 5 <sup>th</sup> layer protective layer   | Acid-treated gelatin<br>Matting agent (z)                 | 490<br>10                          |
|    | 4 <sup>th</sup> layer intermediate layer | Lime-treated gelatin<br>Hardener (ac)                     | 240<br>250                         |
|    | 3 <sup>rd</sup> layer solvent layer      | Lime-treated gelatin<br>Solvent for silver<br>halide (ah) | 4890<br>5770                       |
| 65 | 2 <sup>nd</sup> layer intermediate layer | Lime-treated gelatin<br>Hardener (ac)                     | 370<br>500                         |

TABLE 5-continued

| Construction of processing material P-2 |                                  |                                    |
|-----------------------------------------|----------------------------------|------------------------------------|
| Layer construction                      | Materials added                  | Amounts added (mg/m <sup>2</sup> ) |
| 1 <sup>st</sup> layer primer layer      | Lime-treated gelatin             | 247                                |
|                                         | Water soluble polymer (v)        | 12                                 |
|                                         | Surfactant (r)                   | 14                                 |
|                                         | Hardener (ac)                    | 178                                |
|                                         | Transparent support (63 $\mu$ m) |                                    |



### Hardener (t)



Water-soluble polymer (v):  $\kappa$ -carrageenan

Water-soluble polymer (w): Sumikagel L-5H  
(manufactured by Sumitomo Chemical Co., Ltd.)



Matting Agent (z): SYLOID 79 (manufactured by Fuji-Davison Chemical Co., Ltd.)



Organic solvent having a high boiling point (af): EMPARA K65 (manufactured by Ajinomoto Co., Ltd.)



Photosensitive materials 102 to 113 were prepared by the same procedure for preparation of layers as that of the photosensitive material 101, except that the cyan dye and the surfactant for use as dispersant of the solid dispersion of the cyan dye in the antihalation layer of the photosensitive material 101 were changed according to Table 6.

TABLE 6

| Additive (x)   | 1 <sup>st</sup> layer (antihalation layer) |                                                                |                                                             |            |
|----------------|--------------------------------------------|----------------------------------------------------------------|-------------------------------------------------------------|------------|
|                | Photo-sensitive material                   | Decolorizing dye No. (coating weight of dye g/m <sup>2</sup> ) | Dispersant (coating weight of dispersant g/m <sup>2</sup> ) |            |
| 55             | 101                                        | F-81 (0.132 g/m <sup>2</sup> )                                 | Surfactant (p) (0.012)                                      | Example 1  |
|                | 102                                        | F-47 (0.105)                                                   | Surfactant (p) (0.009)                                      | Example 2  |
|                | 103                                        | F-49 (0.121)                                                   | Surfactant (p) (0.011)                                      | Example 3  |
|                | 104                                        | F-50 (0.115)                                                   | Surfactant (p) (0.010)                                      | Example 4  |
|                | 60                                         | 105 F-3 (0.100)                                                | Surfactant (p) (0.009)                                      | Example 5  |
|                | 106                                        | F-85 (0.147)                                                   | Surfactant (p) (0.013)                                      | Example 6  |
|                | 107                                        | F-116 (0.129)                                                  | Surfactant (p) (0.012)                                      | Example 7  |
|                | 108                                        | F-117 (0.136)                                                  | Surfactant (p) (0.012)                                      | Example 8  |
| Surfactant (y) | 109                                        | F-81 (0.132)                                                   | Surfactant (c-1) (0.012)                                    | Example 9  |
|                | 110                                        | F-81 (0.132)                                                   | Surfactant (c-2) (0.012)                                    | Example 10 |
|                | 65                                         | 111 F-81 (0.132)                                               | Sodium dodecylbenzenesulfonate (0.012)                      | Example 11 |

TABLE 6-continued

| 1 <sup>st</sup> layer (antihalation layer) |                                                                |                                                             |            |
|--------------------------------------------|----------------------------------------------------------------|-------------------------------------------------------------|------------|
| Photo-sensitive material                   | Decolorizing dye No. (coating weight of dye g/m <sup>2</sup> ) | Dispersant (coating weight of dispersant g/m <sup>2</sup> ) |            |
| 112                                        | F-50 (0.115)                                                   | Surfactant (c-1) (0.010)                                    | Example 12 |
| 113                                        | F-50 (0.115)                                                   | Surfactant (c-2) (0.010)                                    | Example 13 |



x/y=70/30 (molar ratio); number average molecular weight: 5,300



x/y=55/45

#### Comparative Examples 1 to 3

Photosensitive materials H-1 and H-2 were prepared by the same procedure for preparation of layers as that of the photosensitive material 101, except that the cyan dye in the antihalation layer of the photosensitive material 101 was changed according to Table 7. The cyan dye (ai) of H-2 was added as an emulsified dispersion of the cyan dye (ai).

The emulsified dispersion was prepared by the same procedure as that of the preparation of the emulsified dispersion of dye for the yellow filter layer, except that 7.1 g of the yellow dye (1) was replaced by 14.2 g of the following cyan dye (ai) and 7.1 g of the organic solvent having a high boiling point was replaced by 14.2 g of the following organic solvent having a high boiling point (C-3).

Further, photosensitive materials H-3 was prepared by the same procedure for preparation of layers as that of the photosensitive material 101 of the photosensitive material 101, except that the cyan dye in the antihalation layer was replaced by black colloidal silver as shown in Table 7.

TABLE 7

| 1 <sup>st</sup> layer (antihalation layer) |                                                                                 |                                                             |                       |
|--------------------------------------------|---------------------------------------------------------------------------------|-------------------------------------------------------------|-----------------------|
| Photo-sensitive material                   | Decolorizing dye (coating weight of dye g/m <sup>2</sup> )                      | Dispersant (coating weight of dispersant g/m <sup>2</sup> ) |                       |
| H-1                                        | No dye used                                                                     | —                                                           | Comparative example 1 |
| H-2                                        | Compound (ai) (0.158)                                                           | Sodium dodecylbenzenesulfonate (0.014)                      | Comparative example 2 |
| H-3                                        | Black colloidal silver (coating weight based on silver: 0.24 g/m <sup>2</sup> ) | —                                                           | Comparative example 3 |



15 mL/m<sup>2</sup> of water (equivalent of 45% of the amount required for maximum swelling) of 40° C. was supplied to the photosensitive materials 101 to 113 and H-1 to H-3, without being exposed to light. Then, these photosensitive materials were each put together with the processing material P-1 and heated from the back face of the photosensitive material by a heat drum of 83° C. for 17 seconds. After that, the processing material P-1 was peeled from the photosensitive material. Again, 15 mL/m<sup>2</sup> of water of 40° C. was supplied to the photosensitive material. Then, the photosensitive material was put together with the processing material P-2 and heated at 83° C. for 10 seconds. The processing material P-2 was then peeled from the photosensitive material. The photosensitive materials thus obtained were subjected to the measurement of transmitted density by status filter A. The measurement was conducted at 3 points and the averages are shown as results in Table 8.

As is apparent from the results shown in Table 8, since Dmin of the photosensitive materials of the present invention after processing is equivalent to that of the photosensitive material H-1 (Comparative Example 1) containing no dye, the photosensitive materials of the present invention, in which the decolorizing dye having the structure represented by the general formula (I) and silver are present in the same layer, are so excellent in decolorizing property that the color is completely lost by the processing.

In addition, the photosensitive materials 101 to 113 and H-1 to H-3, without being exposed to light, were developed

by using a liquid developer (CN-16) manufactured by Fuji Photo Film Co., Ltd. and the photosensitive materials thus obtained were subjected to the evaluation of  $D_{min}$  according to the same method as that described above. As is apparent from the results shown in Table 8, the photosensitive materials of the present invention have excellent decolorizing property also in development by the liquid developer as in heat development.

The photosensitive material thus prepared was cut into APS format, punched, and loaded in a cartridge, which was

5 images were processed in the same way as above and the quality (sharpness and color reproduction) of the images was evaluated. The results were expressed by  $\circ$  and  $\times$  based on the same criterion as above.

Further, the photosensitive materials of the present invention were left for aging in a condition of 45° C. and 80% humidity for 3 days. After that, the photosensitive materials were processed (2 kinds, i.e., heat development and liquid development) and evaluated in the same way. The results are shown in Table 8.

TABLE 6

| Examples                      |                       | Dmin transmitted density (status A filter) |                 |                |                        |                    |                 |                |                        | Evaluation results of print images |                            |                   |                            |
|-------------------------------|-----------------------|--------------------------------------------|-----------------|----------------|------------------------|--------------------|-----------------|----------------|------------------------|------------------------------------|----------------------------|-------------------|----------------------------|
|                               |                       | Heat development                           |                 |                |                        | Liquid development |                 |                |                        | After 3 days                       |                            | After 3 days      |                            |
| Photo- and sensitive material | Comparative Examples  | Cyan density                               | Magenta density | Yellow density | De-colorizing property | Cyan density       | Magenta density | Yellow density | De-colorizing property | Before aging test                  | at 45° C. and 80% humidity | Before aging test | at 45° C. and 80% humidity |
|                               |                       | 101 Example 1                              | 0.51            | 0.62           | 1.12                   | ○                  | 0.28            | 0.84           | 1.05                   | ○                                  | ○                          | ○                 | ○                          |
| 102                           | Example 2             | 0.49                                       | 0.63            | 1.15           | ○                      | 0.27               | 0.85            | 1.04           | ○                      | ○                                  | ○                          | ○                 | ○                          |
| 103                           | Example 3             | 0.52                                       | 0.60            | 1.13           | ○                      | 0.26               | 0.86            | 1.05           | ○                      | ○                                  | ○                          | ○                 | ○                          |
| 104                           | Example 4             | 0.52                                       | 0.62            | 1.10           | ○                      | 0.24               | 0.87            | 1.03           | ○                      | ○                                  | ○                          | ○                 | ○                          |
| 105                           | Example 5             | 0.53                                       | 0.63            | 1.15           | ○                      | 0.26               | 0.84            | 1.02           | ○                      | ○                                  | ○                          | ○                 | ○                          |
| 106                           | Example 6             | 0.48                                       | 0.60            | 1.12           | ○                      | 0.24               | 0.85            | 1.03           | ○                      | ○                                  | ○                          | ○                 | ○                          |
| 107                           | Example 7             | 0.50                                       | 0.61            | 1.13           | ○                      | 0.25               | 0.86            | 1.04           | ○                      | ○                                  | ○                          | ○                 | ○                          |
| 108                           | Example 8             | 0.51                                       | 0.63            | 1.12           | ○                      | 0.24               | 0.86            | 1.05           | ○                      | ○                                  | ○                          | ○                 | ○                          |
| 109                           | Example 9             | 0.48                                       | 0.61            | 1.14           | ○                      | 0.26               | 0.86            | 1.04           | ○                      | ○                                  | ○                          | ○                 | ○                          |
| 110                           | Example 10            | 0.52                                       | 0.62            | 1.15           | ○                      | 0.25               | 0.85            | 1.04           | ○                      | ○                                  | ○                          | ○                 | ○                          |
| 111                           | Example 11            | 0.52                                       | 0.60            | 1.12           | ○                      | 0.26               | 0.84            | 1.03           | ○                      | ○                                  | ○                          | ○                 | ○                          |
| 112                           | Example 12            | 0.49                                       | 0.62            | 1.14           | ○                      | 0.27               | 0.85            | 1.05           | ○                      | ○                                  | ○                          | ○                 | ○                          |
| 113                           | Example 13            | 0.48                                       | 0.61            | 1.12           | ○                      | 0.26               | 0.85            | 1.02           | ○                      | ○                                  | ○                          | ○                 | ○                          |
| H-1                           | Comparative example 1 | 0.48                                       | 0.59            | 1.05           | Reference standard     | 0.25               | 0.81            | 1.01           | Reference standard     | ×                                  | ×                          | ×                 | ×                          |
| H-2                           | Comparative example 2 | 0.46                                       | 0.60            | 1.10           | ○                      | 1.21               | 0.90            | 1.05           | ×                      | ○                                  | ○                          | ○                 | ○                          |
| H-3                           | Comparative example 3 | 1.22                                       | 1.10            | 1.60           | ×                      | 0.32               | 0.85            | 1.08           | ○                      | ○                                  | ○                          | ○                 | ○                          |

then loaded in an APS camera. In this way, photographs of a person and a Macbeth chart were taken by using the 50 photosensitive material.

From this photosensitive material thus exposed was processed using the processing materials P-1 and P-2 in the above-described way to thereby obtain a negative image on the photosensitive material. The image was read out by a 55 digital image scanner, "Frontier SP-1000" manufactured by Fuji Photo Film Co., Ltd., and image-processed in work station. After that, a print image was obtained by a heat-development printer ("Pictography" 4000 manufactured by Fuji Photo Film Co., Ltd.). The quality of print images was evaluated, and the results are shown in Table 8 according to the following rating:  $\circ$ : sharpness and color reproduction are excellent;  $\times$ : sharpness and color reproduction are poor or defects such as halation are observed.

Negative images were obtained from the photosensitive 65 materials exposed in the same way as above but by development using a liquid developer (CN-16). The negative

The following can be seen from the results of Table 8.

50 In the print image obtained from the photosensitive material H-1 of Comparative Example 1, the edges of image having cyan density were not sharp. This indicates that antihalation effect is not sufficient. As in the photosensitive material H-2 of Comparative Example 2, the edges of image become sharp if the cyan dye (ai) is used in the antihalation layer. However, the problem of the photosensitive material H-2 is that the decolorizing property after liquid development is insufficient and unnecessary color components remain when image data are read out. Further, as in the photosensitive material H-3 of Comparative Example 3, the 60 edges of image become sharp if black colloidal silver is used in the antihalation layer. However, the problem of the photosensitive material H-2 is that the decolorizing property after heat development is insufficient and unnecessary color components remain. To the contrary, in the photosensitive materials 101 to 113 of the present invention in Examples 1 to 13, the halation preventing effect is so sufficient that no unnecessary color components remain either after heat

development or liquid development. Furthermore, images having the same sharpness can be obtained both before and after the storage test, thus indicating good decolorizing property of the photosensitive materials of the present invention.

Although Examples described above provide examples in which the dye represented by the general formula (I) is incorporated in a non-photosensitive layer, it goes without saying that the same effect is obtained also in the case where the dye is incorporated in a photosensitive layer.

The present invention provides a silver halide color photographic photosensitive material incorporated with a color developing agent and a coupler, characterized in that the decolorizing property of dye is so excellent in simple development that any unnecessary color component does not remain when color information is read out and in that images excellent in color separation and sharpness can be obtained even after the storage of the photosensitive material. Further, the present invention provides an image forming method using the silver halide color photographic photosensitive material.

What is claimed is:

1. A method of forming an image, comprising the steps of:

(a) providing a silver halide color photographic photosensitive material which comprises:  
a support having thereon a photosensitive silver halide emulsion layer containing photosensitive silver halide grains, a color developing agent, a coupler and a binder, and a non-photosensitive layer, and  
an antihalation layer formed between the silver halide emulsion layer and the support, or on a surface of the support at a side thereof opposite to a side thereof on which the silver halide emulsion layer is provided, wherein an antihalation dye is contained as a dispersion of solid fine particles in the antihalation layer, the dye being selected from at least one of the group consisting of (I-7) and



wherein  $A^{21}$  and  $A^{31}$  each represents 2-pyrazoline-5-one, iso-oxazoline, hydroxypyridine, pyrazolidine-dione, or barbituric acid;  $L^{21}$ ,  $L^{22}$  and  $L^{23}$  each represents a methine group;  $R^{21}$ ,  $R^{22}$ ,  $R^{31}$  and  $R^{32}$  each represents an alkyl or aryl group;  $R^{23}$ ,  $R^{24}$ ,  $R^{25}$ ,  $R^{26}$ ,  $R^{33}$ ,  $R^{34}$ ,  $R^{35}$  and  $R^{36}$  each represents a hydrogen atom or a substituent group; and  $r$  represents an integer selected from the group consisting of 0, 1 and 2, wherein  $R^{23}$  and  $R^{24}$ ,  $R^{21}$  and  $R^{23}$ ,  $R^{21}$  and  $R^{22}$ ,  $R^{22}$  and  $R^{25}$ ,  $R^{25}$  and  $R^{26}$ ,  $R^{23}$  and  $R^{34}$ ,  $R^{31}$  and  $R^{33}$ ,  $R^{31}$  and  $R^{32}$ ,  $R^{32}$  and  $R^{35}$ , and  $R^{35}$  and  $R^{36}$  may optionally form a ring; and

(b) exposing imagewise the silver halide color photographic photosensitive material; and

(c) developing, contemporaneously with or after the step of exposing, the silver halide color photographic photosensitive material in the presence of a decolorizing agent or a precursor thereof,

wherein said dye has a dissociative proton or a group having a dissociative proton, which is linked to said dye directly or via a divalent linking group.

5 10 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845

- a compound capable of performing a complex forming reaction with a metal ion resulting from said basic metal compound;
- (c) placing the processing material together with the photosensitive layer thereon facing the processing layer;
- (d) swelling the layers by adding water, wherein the amount of water ranges from the minimum amount required for maximum swelling, excluding layers that function only as backing, to  $\frac{1}{10}$  of said minimum; and
- (e) heating from 1 to 120 seconds to achieve a temperature ranging from 50 to 100° C. in the photosensitive layer and processing layer,
- wherein said dye has a dissociative proton or a group having a dissociative proton, which is linked to said dye directly or via a divalent linking group.

6. The method of forming an image according to claim 1, wherein said decolorizing agent is alcohol or phenols ( $R_{51}OH$ ), amines or anilines ( $(R_{52})_3N$ ), hydroxylamines ( $(R_{52})_2NOR_{52}$ ), sulfonic acids ( $R_{51}SO_2H$ ) or salts thereof, sulfurous acid or salts thereof, thiosulfuric acid or salts thereof, carboxylic acids ( $R_{51}CO_2H$ ) or salts thereof, hydrazines ( $(R_{52})_2NN(R_{52})_2$ ), guanidines ( $((R_{52})_2N)_2C\equiv NH$ ), aminoguanidines ( $((R_{52})_2NR_{52}N(R_{52})N)C\equiv NH$ ), amidines, thiols ( $R_{51}SH$ ), cyclic or chain active methylene compounds ( $Z_{53}—CH_2—Z_{54}$ ), cyclic or chain methylene compounds ( $Z_{53}CH(R_{51})—Z_{54}$ ) or  $Z_{53}—CH(Z_{54})—Z_{55}$ , where  $Z_{55}$  is the same as  $Z_{53}$  and where  $Z_{53}$ ,  $Z_{54}$ , and  $Z_{55}$  (or  $R_{51}$ ) may join with each other to form a ring, and anionic species derived from these compounds; and  $R_{51}$  represents an alkyl group, an alkenyl group, a cycloalkyl group, an aryl group or a heterocyclic group, while  $R_{52}$  represents a hydrogen atom or the same group as  $R_{51}$ , each of  $R_{51}$  and  $R_{52}$  may

have a substituent group, if a plurality of  $R_{51}$  or  $R_{52}$  are present in the molecule, they may be the same or different,  $Z_{53}$  and  $Z_{54}$  are each selected from the group consisting of  $—CN$ ,  $—SO_2R_{51}$ ,  $—COR_{51}$ ,  $—COOR_{51}$ ,  $—CON(R_{52})_2$ ,  $—SO_2N(R_{52})_2$ ,  $—C\equiv C(CN)_2R_{51}$  and  $—C\equiv C(CN)_2N(R_{51})_2$  wherein  $Z_{53}$  may be the same as or different from  $Z_{54}$ , and  $Z_{53}$  and  $Z_{54}$  may join together to form a ring.

7. The method of forming an image according to claim 5, wherein said decolorizing agent is alcohol, phenols ( $R_{51}OH$ ), amines, anilines ( $(R_{52})_3N$ ), hydroxylamines ( $(R_{52})_2NOR_{52}$ ), sulfonic acids ( $R_{51}SO_2H$ ) or salts thereof, sulfurous acid or salts thereof, thiosulfuric acid or salts thereof, carboxylic acids ( $R_{51}CO_2H$ ) or salts thereof, hydrazines ( $(R_{52})_2NN(R_{52})_2$ ), guanidines ( $((R_{52})_2N)_2C\equiv NH$ ), aminoguanidines ( $((R_{52})_2NR_{52}N(R_{52})N)C\equiv NH$ ), amidines, thiols ( $R_{51}SH$ ), cyclic or chain active methylene compounds ( $Z_{53}—CH_2—Z_{54}$ ), cyclic or chain methylene compounds ( $Z_{53}CH(R_{51})—Z_{54}$ ) or  $Z_{53}—CH(Z_{54})—Z_{55}$ , where  $Z_{55}$  is the same as  $Z_{53}$  and where  $Z_{53}$ ,  $Z_{54}$ , and  $Z_{55}$  (or  $R_{51}$ ) may join with each other to form a ring, and anionic species derived from these compounds; and  $R_{51}$  represents an alkyl group, an alkenyl group, a cycloalkyl group, an aryl group or a heterocyclic group, while  $R_{52}$  represents a hydrogen atom or the same group as  $R_{51}$ , each of  $R_{51}$  and  $R_{52}$  may have a substituent group; if a plurality of  $R_{51}$  or  $R_{52}$  are present in the molecule, they may be the same or different;  $Z_{53}$  and  $Z_{54}$  are each selected from the group consisting of  $—CN$ ,  $—SO_2R_{51}$ ,  $—COR_{51}$ ,  $—COOR_{51}$ ,  $—CON(R_{52})_2$ ,  $—SO_2N(R_{52})_2$ ,  $—C\equiv C(CN)_2R_{51}$  and  $—C\equiv C(CN)_2N(R_{51})_2$  wherein  $Z_{53}$  may be the same as or different from  $Z_{54}$ , and  $Z_{53}$  and  $Z_{54}$  may optionally join together to form a ring.

\* \* \* \* \*